



US008444776B1

(12) **United States Patent**  
**Bailey et al.**

(10) **Patent No.:** **US 8,444,776 B1**  
(b4) **Date of Patent:** **May 21, 2013**

(54) **HIGH HARDNESS, HIGH TOUGHNESS IRON-BASE ALLOYS AND METHODS FOR MAKING SAME**

(75) Inventors: **Ronald E. Bailey**, Pittsburgh, PA (US); **Thomas R. Parayil**, New Kensington, PA (US); **Glenn J. Swiatek**, Palos Heights, IL (US)

(73) Assignee: **ATI Properties, Inc.**, Albany, OR (US)

(\*) Notice: Subject to any disclaimer, the term of this patent is extended or adjusted under 35 U.S.C. 154(b) by 631 days.

(21) Appl. No.: **12/581,497**

(22) Filed: **Oct. 19, 2009**

**Related U.S. Application Data**

(63) Continuation-in-part of application No. 12/184,573, filed on Aug. 1, 2008.

(60) Provisional application No. 60/953,269, filed on Aug. 1, 2007.

(51) **Int. Cl.**  
**C22C 38/44** (2006.01)

(52) **U.S. Cl.**  
USPC ..... **148/335; 420/108**

(58) **Field of Classification Search**  
USPC ..... 148/335; 420/108  
See application file for complete search history.

(56) **References Cited**

**U.S. PATENT DOCUMENTS**

1,016,560 A 2/1912 Giolitti  
1,563,420 A 12/1925 Johnson  
2,562,467 A 7/1951 Kinnear, Jr.

3,379,582 A 4/1968 Dickinson  
3,785,801 A 1/1974 Benjamin  
3,888,637 A 6/1975 Taguchi et al.  
4,443,254 A 4/1984 Floreen  
4,484,959 A 11/1984 Boucher et al.  
4,645,720 A 2/1987 Pircher et al.  
4,788,034 A 11/1988 Brandis et al.  
4,832,909 A 5/1989 Schmidt et al.  
4,871,511 A 10/1989 Smith, Jr. et al.  
4,941,927 A 7/1990 Hickey, Jr. et al.  
5,122,336 A 6/1992 Roux et al.  
5,129,966 A \* 7/1992 Rao ..... 148/542  
5,268,044 A 12/1993 Hemphill et al.  
5,332,545 A 7/1994 Love

(Continued)

**FOREIGN PATENT DOCUMENTS**

DE A-41 07 417 12/1991  
DE 4344879 A1 7/1995

(Continued)

**OTHER PUBLICATIONS**

ATI 600-MIL® Ultra High Hard Specialty Armor; Version 4; Aug. 10, 2010.

(Continued)

*Primary Examiner* — Jie Yang

(74) *Attorney, Agent, or Firm* — K & L Gates LLP; Patrick J. Viccaro; John E. Grosselin, III

(57) **ABSTRACT**

An aspect of the present disclosure is directed to low-alloy steels exhibiting high hardness and an advantageous level of multi-hit ballistic resistance with low or no crack propagation imparting a level of ballistic performance suitable for military armor applications. Various embodiments of the steels according to the present disclosure have hardness in excess of 550 BHN and demonstrate a high level of ballistic penetration resistance relative to conventional military specifications.

**13 Claims, 17 Drawing Sheets**



## U.S. PATENT DOCUMENTS

|                 |        |                 |
|-----------------|--------|-----------------|
| 5,720,829 A     | 2/1998 | Finkl et al.    |
| 5,749,140 A     | 5/1998 | Polito et al.   |
| 5,866,066 A     | 2/1999 | Hemphill et al. |
| 6,080,359 A     | 6/2000 | Davidson        |
| 6,087,013 A     | 7/2000 | Chilson         |
| 6,360,936 B1    | 3/2002 | Dilg et al.     |
| 6,361,883 B1    | 3/2002 | Dilg et al.     |
| 7,981,521 B2    | 7/2011 | Bailey et al.   |
| 2011/0067788 A1 | 3/2011 | Swiatek et al.  |
| 2001/0236721    | 9/2011 | Bailey et al.   |

## FOREIGN PATENT DOCUMENTS

|    |                   |         |
|----|-------------------|---------|
| EP | 051401 A1         | 5/1982  |
| EP | 327042 A1         | 8/1989  |
| EP | 0731332 A2        | 9/1996  |
| EP | 1111325 A2        | 6/2001  |
| EP | 2036992 A1        | 3/2009  |
| FR | 2106939           | 5/1972  |
| GB | 874488            | 8/1961  |
| GB | 2 054 110         | 7/1979  |
| GB | 763442            | 4/1982  |
| JP | S49-9899 A        | 1/1974  |
| JP | 57-83575 A        | 5/1982  |
| JP | 58-157950 A       | 9/1983  |
| JP | 58-199846 A       | 11/1983 |
| JP | 59-6356 A         | 1/1984  |
| JP | 60-29446 A        | 2/1985  |
| JP | H01-296098 A      | 11/1989 |
| JP | 57-161049 A       | 10/2002 |
| SU | 404889            | 10/1973 |
| WO | WO 2004/111277 A1 | 12/2004 |
| WO | WO 2009/018522 A1 | 2/2009  |

## OTHER PUBLICATIONS

ATI 500-MIL® High Hard Specialty Armor; Version 5; Aug. 10, 2010.  
 ATI-K12®-MIL Dual Hard Armor Plate; Version 3; Sep. 10, 2009.  
 ATI-K12®-MIL Dual Hard Armor Plate; Version 4; Aug. 10, 2010.  
 Military Specification MIL-A-12560H (MR); Nov. 28, 1990.  
 Military Specification MIL-DTL-32332 (MR); Jul. 24, 2009.

Military Specification MIL-DTL-46100E (MR); Jul. 9, 2008.  
 Military Specification MIL-DTL-12560J (MR); Jul. 24, 2009.  
 Military Specification MIL-A-45099C; Sep. 14, 1987.  
 Military Specification MIL-A-46100D (MR) with int. amendment 2; Jul. 13, 2007.  
 ASTM International, Standard Specification for Steel Bars, Designation; A29/A29M-05, Carbon and Alloy, Hot Wrought, General Requirements for, 2005, pp. 1-16.  
 Alloy Digest, Data on World Wide Metals and Alloys, AISI 4820 (Nickel-Molybdenum Carburizing Steel), Nov. 1974. 2 pages.  
 Data Sheet entitled VascoMax T-200/T-250/T-300 Teledyne Vasco 1985, pp. 2-11.

U.S. Appl. No. 12/184,573, filed Aug. 1, 2008.  
 U.S. Appl. No. 12/986,213, filed Jan. 7, 2011.  
 Definition of "cross rolling", The Metals Handbook Desk Edition, 2nd Edition, published by ASM International of Metals Park, Ohio, 1996, p. 17.  
 Sulfide Inclusions in Steel, Proceedings of an International Symposium. Nov. 7-8, 1974, Port Chester, New York, pp. 206, 255-256.  
 Metals Handbook, Tenth Edition, vol. 1, Properties and Selection: Irons, Steels, and High-Performance Alloys, J.R. Davis, editor, published by ASM International, Materials Park, OH, 1990, p. 400.  
 DeArdo and E.G. Hamburg: "Influence of Elongated Inclusions on the Mechanical Properties of High Strength Steel Plate," Sulfide Inclusions in Steel, J.J. de Barbadillo and E. Snape, ed., American Society for Metals, Metals Park, OH, 1975. pp. 309-337; 359.  
 ARMOX(TM) 600T (ARMOX 600S) Data Sheet, SSAB Oxelösund AB, Jun. 6, 2006.  
 "K12(R) Dual Hardness Armor Plate" Technical Data Sheet, Allegheny Ludlum, 2002.  
 "Allegheny Ludlum AL 600(TM) (UNS Designation N6600) Nickel-Base Alloy," Allegheny Ludlum Corporation, Pittsburgh, PA, 1998.  
 C.F. Hickey, et al., "Comparing a Split Heat of ESR/VAR 4340 Steel," Metal Progress, Oct. 1985, pp. 69-74.  
 "Steels Double Up for Composites," The Iron Age, Nov. 16, 1967, pp. 70-72.  
 "Review of Recent Armor Plate Developments" by Rathbone, Blast Furnace and Steel Plant, Jul. 1968, pp. 575-583.

\* cited by examiner

**FIG. 1**

Panel variable: Gage



FIG. 2



FIG. 3

Panel variables: Quench, Gage

**FIG. 4**

79804AB3



79804AB1

**FIG. 5**



FIG. 6

**FIG. 7**



FIG. 8



FIG. 9



FIG. 10



FIG. 11



FIG. 12



FIG. 13



FIG. 14

**FIG. 15**



**FIG. 16**

**FIG. 17**

**FIG. 18**

**FIG. 19**

10050491

3

5

1

6

4

2

**FIG. 20**

## HIGH HARDNESS, HIGH TOUGHNESS IRON-BASE ALLOYS AND METHODS FOR MAKING SAME

### CROSS-REFERENCE TO RELATED APPLICATIONS

The present application is a continuation-in-part of U.S. patent application Ser. No. 12/184,573, filed on Aug. 1, 2008. U.S. patent application Ser. No. 12/184,573 claims priority under 35 U.S.C. §119(e) to U.S. Provisional Patent Application Ser. No. 60/953,269, filed Aug. 1, 2007. U.S. patent application Ser. Nos. 12/184,573 and 60/953,269 are incorporated by reference herein.

### TECHNICAL FIELD

The present disclosure relates to iron-base alloys having hardness greater than 550 BHN (Brinell hardness number) and demonstrating substantial and unexpected penetration resistance and crack resistance in standard ballistic testing. The present disclosure also relates to armor and other articles of manufacture including the alloys. The present disclosure further relates to methods of processing various iron-base alloys so as to improve resistance to ballistic penetration and cracking.

### BACKGROUND

Armor plate, sheet, and bar are commonly provided to protect structures against forcibly launched projectiles. Although armor plate, sheet, and bar are typically used in military applications as a means to protect personnel and property within, for example, vehicles and mechanized armaments, the products also have various civilian uses. Such uses may include, for example, sheathing for armored civilian vehicles and blast-fortified property enclosures. Armor has been produced from a variety of materials including, for example, polymers, ceramics, and metallic alloys. Because armor is often mounted on mobile articles, armor weight is typically an important factor. Also, the costs associated with producing armor can be substantial, and particularly so in connection with exotic armor alloys, ceramics, and specialty polymers. As such, an objective has been to provide lower-cost yet effective alternatives to existing armors, and without significantly increasing the weight of armor necessary to achieve the desired level of ballistic performance (penetration resistance and cracking resistance).

Also, in response to ever-increasing anti-armor threats, the United States military had for many years been increasing the amount of armor used on tanks and other combat vehicles, resulting in significantly increased vehicle weight. Continuing such a trend could drastically adversely affect transportability, portable bridge-crossing capability, and maneuverability of armored combat vehicles. Within the past decade the U.S. military has adopted a strategy to be able to very quickly mobilize its combat vehicles and other armored assets to any region in the world as the need may arise. Thus, concern over increasing combat vehicle weight has taken center stage. As such, the U.S. military has been investigating a number of possible alternative, lighter-weight armor materials, such as certain titanium alloys, ceramics, and hybrid ceramic tile/polymer-matrix composites (PMCs).

Examples of common titanium alloy armors include Ti-6Al-4V, Ti-6Al-4V ELI, and Ti-4Al-2.5V—Fe—O. Titanium alloys offer many advantages relative to more conventional rolled homogenous steel armor. Titanium alloys have a

high mass efficiency compared with rolled homogenous steel and aluminum alloys across a broad spectrum of ballistic threats, and also provide favorable multi-hit ballistic penetration resistance capability. Titanium alloys also exhibit generally higher strength-to-weight ratios, as well as substantial corrosion resistance, typically resulting in lower asset maintenance costs. Titanium alloys may be readily fabricated in existing production facilities, and titanium scrap and mill revert can be remelted and recycled on a commercial scale.

10 Nevertheless, titanium alloys do have disadvantages. For example, a spall liner typically is required, and the costs associated with manufacturing the titanium armor plate and fabricating products from the material (for example, machining and welding costs) are substantially higher than for rolled homogenous steel armors.

15 Although PMCs offer some advantages (for example, freedom from spalling against chemical threats, quieter operator environment, and high mass efficiency against ball and fragment ballistic threats), they also suffer from a number of disadvantages. For example, the cost of fabricating PMC components is high compared with the cost for fabricating components from rolled homogenous steel or titanium alloys, and PMCs cannot readily be fabricated in existing production facilities. Also, non-destructive testing of PMC materials may 20 not be as well advanced as for testing of alloy armors. Moreover, multi-hit ballistic penetration resistance capability and automotive load-bearing capacity of PMCs can be adversely affected by structural changes that occur as the result of an initial projectile strike. In addition, there may be a fire and fume hazard to occupants in the interior of combat vehicles covered with PMC armor, and PMC commercial manufacturing and recycling capabilities are not well established.

25 Metallic alloys are often the material of choice when selecting an armor material. Metallic alloys offer substantial multi-hit protection, typically are inexpensive to produce relative to exotic ceramics, polymers, and composites, and may be readily fabricated into components for armored combat vehicles and mobile armament systems. It is conventionally believed that it is advantageous to use materials having 30 very high hardnesses in armor applications because projectiles are more likely to fragment when impacting higher hardness materials. Certain metallic alloys used in armor application may be readily processed to high hardnesses, typically by quenching the alloys from very high temperatures.

35 45 Because rolled homogenous steel alloys are generally less expensive than titanium alloys, substantial effort has focused on modifying the composition and processing of existing rolled homogenous steels used in armor applications since even incremental improvements in ballistic performance are significant. For example, improved ballistic threat performance can allow for reduced armor plating thicknesses without loss of function, thereby reducing the overall weight of an armor system. Because high system weight is a primary drawback of metallic alloy systems relative to, for example, polymer and ceramic armors, improving ballistic threat performance can make alloy armors more competitive relative to exotic armor systems.

40 50 55 Over the last 25 years, relatively light-weight clad and composite steel armors have been developed. Certain of these composite armors, for example, combine a front-facing layer of high-hardness steel metallurgically bonded to a tough, penetration resistant steel base layer. The high-hardness steel layer is intended to break up the projectile, while the tough underlayer is intended to prevent the armor from cracking, shattering, or spalling. Conventional methods of forming a composite armor of this type include roll bonding stacked plates of the two steel types. One example of a composite

armor is K12® armor plate, which is a dual hardness, roll-bonded composite armor plate available from ATI Allegheny Ludlum, Pittsburgh, Pa. K12® armor plate includes a high hardness front side and a softer back side. Both faces of the K12® armor plate are Ni—Mo—Cr alloy steel, but the front side includes higher carbon content than the back side. K12® armor plate has superior ballistic performance properties compared to conventional homogenous armor plate and meets or exceeds the ballistic requirements for numerous government, military, and civilian armoring applications. Although clad and composite steel armors offer numerous advantages, the additional processing involved in the cladding or roll bonding process necessarily increases the cost of the armor systems.

Relatively inexpensive low alloy content steels also are used in certain armor applications. As a result of alloying with carbon, chromium, molybdenum, and other elements, and the use of appropriate heating, quenching, and tempering steps, certain low alloy steel armors can be produced with very high hardness properties, greater than 550 BHN. Such high hardness steels are commonly known as "600 BHN" steels. Table 1 provides reported compositions and mechanical properties for several examples of available 600 BHN steels used in armor applications. MARS 300 and MARS 300 Ni+ are produced by the French company Arcelor. ARMOX 600T armor is available from SSAB Oxelosund AB, Sweden. Although the high hardness of 600 BHN steel armors is very effective at breaking up or flattening projectiles, a significant disadvantage of these steels is that they tend to be rather brittle and readily crack when ballistic tested against, for example, armor piercing projectiles. Cracking of the materials can be problematic to providing multi-hit ballistic resistance capability.

TABLE 1

| Alloy           | C             | Mn           | P<br>(max) | S<br>(max) | Si          | Cr            | Ni           | Mn               | Yield<br>Strength<br>(MPa) | Tensile<br>Strength<br>(MPa) | Elong.<br>(%) | BHN<br>(min) |
|-----------------|---------------|--------------|------------|------------|-------------|---------------|--------------|------------------|----------------------------|------------------------------|---------------|--------------|
| Mars 300        | 0.45-<br>0.55 | 0.3-<br>0.7  | 0.012      | 0.005      | 0.6-<br>1.0 | 0.4<br>(max)  | 4.5<br>(max) | 0.3-<br>0.5      | ≥1,300                     | ≥2,000                       | ≥6%           | 578-<br>655  |
| Mars 300<br>Ni+ | 0.45-<br>0.55 | 0.3-<br>0.7  | 0.01       | 0.005      | 0.6-<br>1.0 | 0.01-<br>0.04 | 3.5-<br>4.5  | 0.3-<br>0.5      | ≥ 1,300                    | ≥2,000                       | ≥6%           | 578-<br>655  |
| Armox 600       | 0.47<br>(max) | 1.0<br>(max) | 0.010      | 0.005      | 0.1-<br>0.7 | 1.5<br>(max)  | 3.0<br>(max) | 0.7<br>(typical) | 1,500                      | 2,000                        | ≥7%           | 570-<br>640  |

In light of the foregoing, it would be advantageous to provide an improved steel armor material having hardness within the 600 BHN range and having substantial multi-hit ballistic resistance with reduced crack propagation.

## SUMMARY

According to various non-limiting embodiments of the present disclosure, an iron-base alloy is provided having favorable multi-hit ballistic resistance, hardness greater than 550 BHN, and including, in weight percentages based on total alloy weight: 0.40 to 0.53 carbon; 0.15 to 1.00 manganese; 0.15 to 0.45 silicon; 0.95 to 1.70 chromium; 3.30 to 4.30 nickel; 0.35 to 0.65 molybdenum; 0.0002 to 0.0050 boron; 0.001 to 0.015 cerium; 0.001 to 0.015 lanthanum; no greater than 0.002 sulfur; no greater than 0.015 phosphorus; no greater than 0.011 nitrogen; iron; and incidental impurities.

According to various other non-limiting embodiments of the present disclosure, an alloy mill product such as, for example, a plate, a bar, or a sheet, is provided having hardness

greater than 550 BHN and including, in weight percentages based on total alloy weight: 0.40 to 0.53 carbon; 0.15 to 1.00 manganese; 0.15 to 0.45 silicon; 0.95 to 1.70 chromium; 3.30 to 4.30 nickel; 0.35 to 0.65 molybdenum; 0.0002 to 0.0050 boron; 0.001 to 0.015 cerium; 0.001 to 0.015 lanthanum; no greater than 0.002 sulfur; no greater than 0.015 phosphorus; no greater than 0.011 nitrogen; iron; and incidental impurities.

According to various other non-limiting embodiments of the present disclosure, an armor mill product selected from an armor plate, an armor bar, and an armor sheet is provided having hardness greater than 550 BHN and a V<sub>50</sub> ballistic limit (protection) value that meets or exceeds performance requirements under specification MIL-DTL-46100E. In various embodiments the armor mill product also has a V<sub>50</sub> ballistic limit value that is at least as great as a V<sub>50</sub> ballistic limit value that is 150 feet-per-second less than the performance requirements under specification MIL-A-46099C with reduced or minimal crack propagation. The mill product is an alloy including, in weight percentages based on total alloy weight: 0.40 to 0.53 carbon; 0.15 to 1.00 manganese; 0.15 to 0.45 silicon; 0.95 to 1.70 chromium; 3.30 to 4.30 nickel; 0.35 to 0.65 molybdenum; 0.0002 to 0.0050 boron; 0.001 to 0.015 cerium; 0.001 to 0.015 lanthanum; no greater than 0.002 sulfur; no greater than 0.015 phosphorus; no greater than 0.011 nitrogen; iron; and incidental impurities.

According to various other non-limiting embodiments of the present disclosure, an armor mill product selected from an armor plate, an armor bar, and an armor sheet is provided having hardness greater than 550 BHN and a V<sub>50</sub> ballistic limit (protection) value that meets or exceeds the Class 1 performance requirements under specification MIL-DTL-32332. In various embodiments the armor mill product also

has a V<sub>50</sub> ballistic limit value that is at least as great as a V<sub>50</sub> ballistic limit value that is 150 feet-per-second less than the Class 2 performance requirements under specification MIL-DTL-32332. The mill product is an alloy including, in weight percentages based on total alloy weight: 0.40 to 0.53 carbon; 0.15 to 1.00 manganese; 0.15 to 0.45 silicon; 0.95 to 1.70 chromium; 3.30 to 4.30 nickel; 0.35 to 0.65 molybdenum; 0.0002 to 0.0050 boron; 0.001 to 0.015 cerium; 0.001 to 0.015 lanthanum; no greater than 0.002 sulfur; no greater than 0.015 phosphorus; no greater than 0.011 nitrogen; iron; and incidental impurities.

Various embodiments according to the present disclosure are directed to a method of making an alloy having favorable multi-hit ballistic resistance with reduced or minimal crack propagation and hardness greater than 550 BHN, and wherein the mill product is an alloy including, in weight percentages based on total alloy weight: 0.40 to 0.53 carbon; 0.15 to 1.00 manganese; 0.15 to 0.45 silicon; 0.95 to 1.70 chromium; 3.30 to 4.30 nickel; 0.35 to 0.65 molybdenum; 0.0002 to 0.0050 boron; 0.001 to 0.015 cerium; 0.001 to 0.015 lanthanum; no

greater than 0.002 sulfur; no greater than 0.015 phosphorus; no greater than 0.011 nitrogen; iron; and incidental impurities. The alloy is austenitized by heating the alloy to a temperature of at least 1450° F. The alloy is then cooled from the austenitizing temperature in a manner that differs from the conventional manner of cooling armor alloy from the austenitizing temperature and which alters the path of the cooling curve of the alloy relative to the path the curve would assume if the alloy were cooled in a conventional manner. Cooling the alloy from the austenitizing temperature may provide the alloy with a  $V_{50}$  ballistic limit value that meets or exceeds the required  $V_{50}$  ballistic limit value under specification MIL-DTL-46100E, and in various embodiments under MIL-DTL-32332 (Class 1).

In various embodiments, cooling the alloy from the austenitizing temperature provides the alloy with a  $V_{50}$  ballistic limit value that is no less than a value that is 150 feet-per-second less than the required  $V_{50}$  ballistic limit value under specification MIL-A-46099C, and in various embodiments under specification MIL-DTL-32332 (Class 2), with reduced or minimal crack propagation. In other words, the  $V_{50}$  ballistic limit value is at least as great as a  $V_{50}$  ballistic limit value 150 feet-per-second less than the required  $V_{50}$  ballistic limit value under specification MIL-A-46099C, and in various embodiments under specification MIL-DTL-32332 (Class 2), with reduced or minimal crack propagation.

According to various non-limiting embodiments of a method according to the present disclosure, the step of cooling the alloy comprises simultaneously cooling multiple plates of the alloy from the austenitizing temperature with the plates arranged in contact with one another.

In various embodiments, an alloy article is austenitized by heating the alloy article to a temperature of at least 1450° F. The alloy article is then cooled from the austenitizing temperature in a conventional manner of cooling steel alloys from the austenitizing temperature. The cooled alloy is then tempered at a temperature in the range 250° F. to 500° F. Cooling the alloy from the austenitizing temperature and tempering may provide the alloy with a  $V_{50}$  ballistic limit value that meets or exceeds the required  $V_{50}$  ballistic limit value under specification MIL-DTL-46100E, and in various embodiments under specification MIL-DTL-32332 (Class 1).

In various embodiments, conventional cooling of the alloy article from the austenitizing temperature and tempering provides the alloy article with a  $V_{50}$  ballistic limit value that is no less than a value that is 150 feet-per-second less than the required  $V_{50}$  ballistic limit value under specification MIL-A-46099C, and in various embodiments under specification MIL-DTL-32332 (Class 2), with reduced, minimal, or zero crack propagation. In other words, the  $V_{50}$  ballistic limit value is at least as great as a  $V_{50}$  ballistic limit value 150 feet-per-second less than the required  $V_{50}$  ballistic limit value under specification MIL-A-46099C, and in various embodiments under specification MIL-DTL-32332 (Class 2).

In various embodiments, the alloy article may be an alloy plate or an alloy sheet. An alloy sheet or an alloy plate may be an armor sheet or an armor plate. Other embodiments of the present disclosure are directed to articles of manufacture comprising embodiments of alloys and alloy articles according to the present disclosure. Such articles of manufacture include, for example, armored vehicles, armored enclosures, and items of armored mobile equipment.

It is understood that the invention disclosed and described herein is not limited to the embodiments disclosed in this Summary.

## BRIEF DESCRIPTION OF THE DRAWINGS

Various characteristics of the non-limiting embodiments disclosed and described herein may be better understood by reference to the accompanying figures, in which:

FIG. 1 is a plot of HRC hardness as a function of austenitizing treatment heating temperature for certain experimental plate samples processed as described hereinbelow;

FIG. 2 is a plot of HRC hardness as a function of austenitizing treatment heating temperature for certain non-limiting experimental plate samples processed as described hereinbelow;

FIG. 3 is a plot of HRC hardness as a function of austenitizing treatment heating temperature for certain non-limiting experimental plate samples processed as described hereinbelow;

FIGS. 4, 5 and 7 are schematic representations of arrangements of test samples used during cooling from austenitizing temperature;

FIG. 6 is a plot of  $V_{50}$  velocity over required minimum  $V_{50}$  velocity (as per MIL-A-46099C) as a function of tempering practice for certain test samples;

FIGS. 8 and 9 are plots of sample temperature over time during steps of cooling of certain test samples from an austenitizing temperature;

FIGS. 10 and 11 are schematic representations of arrangements of test samples used during cooling from austenitizing temperature;

FIGS. 12-14 are graphs plotting sample temperature over time for several experimental samples cooled from austenitizing temperature, as discussed herein; and

FIGS. 15-20 are schematic diagrams illustrating photographs of ballistic test panels formed from a high hardness alloy disclosed and described herein.

The reader will appreciate the foregoing details, as well as others, upon considering the following detailed description of various non-limiting embodiments of alloys, articles, and methods according to the present disclosure. The reader also may comprehend additional details upon implementing or using the alloys, articles, and methods described herein.

## DETAILED DESCRIPTION OF NON-LIMITING EMBODIMENTS

It is to be understood that various descriptions of the disclosed embodiments have been simplified to illustrate only those elements, features, and aspects that are relevant to a clear understanding of the disclosed embodiments, while eliminating, for purposes of clarity, other characteristics, features, aspects, and the like. Persons having ordinary skill in the art, upon considering the present description of the disclosed embodiments, will recognize that other characteristics, features, aspects, and the like may be desirable in a particular implementation or application of the disclosed embodiments. However, because such other characteristics, features, aspects, and the like may be readily ascertained and implemented by persons having ordinary skill in the art upon considering the present description of the disclosed embodiments, and are, therefore, not necessary for a complete understanding of the disclosed embodiments, a description of such characteristics, features, aspects, and the like is not provided herein. As such, it is to be understood that the description set forth herein is merely exemplary and illustrative of the disclosed embodiments and is not intended to limit the scope of the invention as defined solely by the claims.

In the present disclosure, other than where otherwise indicated, all numbers expressing quantities or characteristics are

to be understood as being prefaced and modified in all instances by the term "about." Accordingly, unless indicated to the contrary, any numerical parameters set forth in the following description may vary depending on the desired properties one seeks to obtain in the compositions and methods according to the present disclosure. At the very least, and not as an attempt to limit the application of the doctrine of equivalents to the scope of the claims, each numerical parameter described in the present description should at least be construed in light of the number of reported significant digits and by applying ordinary rounding techniques.

Also, any numerical range recited herein is intended to include all sub-ranges subsumed therein. For example, a range of "1 to 10" is intended to include all sub-ranges between (and including) the recited minimum value of 1 and the recited maximum value of 10, that is, having a minimum value equal to or greater than 1 and a maximum value of equal to or less than 10. Any maximum numerical limitation recited herein is intended to include all lower numerical limitations subsumed therein and any minimum numerical limitation recited herein is intended to include all higher numerical limitations subsumed therein. Accordingly, Applicants reserve the right to amend the present disclosure, including the claims, to expressly recite any sub-range subsumed within the ranges expressly recited herein. All such ranges are intended to be inherently disclosed herein such that amending to expressly recite any such sub-ranges would comply with the requirements of 35 U.S.C. §112, first paragraph, and 35 U.S.C. §132(a).

The grammatical articles "one", "a", "an", and "the", as used herein, are intended to include "at least one" or "one or more", unless otherwise indicated. Thus, the articles are used herein to refer to one or more than one (i.e., to at least one) of the grammatical objects of the article. By way of example, "a component" means one or more components, and thus, possibly, more than one component is contemplated and may be employed or used in an implementation of the described embodiments.

Any patent, publication, or other disclosure material, in whole or in part, that is said to be incorporated by reference herein, is incorporated herein in its entirety, but only to the extent that the incorporated material does not conflict with existing definitions, statements, or other disclosure material expressly set forth in this disclosure. As such, and to the extent necessary, the express disclosure as set forth herein supersedes any conflicting material incorporated herein by reference. Any material, or portion thereof, that is said to be incorporated by reference herein, but which conflicts with existing definitions, statements, or other disclosure material set forth herein is only incorporated to the extent that no conflict arises between that incorporated material and the existing disclosure material. Applicants reserve the right to amend the present disclosure to expressly recite any subject matter incorporated by reference herein.

The present disclosure includes descriptions of various embodiments. It is to be understood that all embodiments described herein are exemplary, illustrative, and non-limiting. Thus, the invention is not limited by the description of the various exemplary, illustrative, and non-limiting embodiments. Rather, the invention is defined solely by the claims, which may be amended to recite any features expressly or inherently described in or otherwise expressly or inherently supported by the present disclosure.

The present disclosure, in part, is directed to low-alloy steels having significant hardness and demonstrating a substantial and unexpected level of multi-hit ballistic resistance with reduced, minimal, or zero cracking and/or crack propa-

gation, which imparts a level of ballistic penetration resistance suitable for military armor applications, for example. Various embodiments of the steels according to the present disclosure exhibit hardness values in excess of 550 BHN and 5 demonstrate a substantial level of ballistic penetration resistance when evaluated as per MIL-DTL-46100E, and also when evaluated per MIL-A-46099C. Various embodiments of the steels according to the present disclosure exhibit hardness values in excess of 570 BHN and demonstrate a substantial 10 level of ballistic penetration resistance when evaluated as per MIL-DTL-32332, Class 1 or Class 2, United States Military Specifications "MIL-DTL-46100E", "MIL-A-46099C", and "MIL-DTL-32332" are incorporated by reference herein.

Relative to certain existing 600 BHN steel armor plate 15 materials, various embodiments of the alloys according to the present disclosure are significantly less susceptible to cracking and penetration when tested against armor piercing ("AP") projectiles. Various embodiments of the alloys also have demonstrated ballistic performance that is comparable 20 to the performance of high-alloy armor materials, such as, for example, K-12® armor plate. The ballistic performance of various embodiments of steel alloys according to the present disclosure was wholly unexpected given, for example, the low alloy content of the alloys and the alloys' relatively 25 moderate hardness compared to conventional 600 BHN steel armor materials.

More particularly, it was unexpectedly observed that although various embodiments of alloys according to the present disclosure exhibit relatively moderate hardnesses 30 (which can be provided by cooling the alloys from austenitizing temperatures at a relatively slow cooling rate or at conventional rates), the samples of the alloys exhibited substantial ballistic performance, which was at least comparable to the performance of K-12® armor plate. This surprising and 35 unobvious discovery runs directly counter to the conventional belief that increasing the hardness of steel armor plate materials improves ballistic performance.

Various embodiments of steels according to the present disclosure include low levels of the residual elements sulfur, 40 phosphorus, nitrogen, and oxygen. Also, various embodiments of the steels may include concentrations of one or more of cerium, lanthanum, and other rare earth metals. Without being bound to any particular theory of operation, the inventors believe that the rare earth additions may act to bind some 45 portion of sulfur, phosphorus, and/or oxygen present in the alloy so that these residuals are less likely to concentrate in grain boundaries and reduce the multi-hit ballistic resistance of the material. It is further believed that concentrating sulfur, phosphorus, and/or oxygen within the steels' grain boundaries 50 may promote intergranular separation upon high velocity impact, leading to material fracture, crack propagation, and possible penetration of the impacting projectile. Various embodiments of the steels according to the present disclosure also include relatively high nickel content, for example 3.30 55 to 4.30 weight percent, to provide a relatively tough matrix, thereby significantly improving ballistic performance. In various embodiments, the nickel content may comprise 3.75 to 4.25 weight percent of the steels disclosed herein.

In various embodiments, the steel alloys disclosed herein 60 may comprise (in weight percentages based on total alloy weight): 0.40 to 0.53 carbon; 0.15 to 1.00 manganese; 0.15 to 0.45 silicon; 0.95 to 1.70 chromium; 3.30 to 4.30 nickel; 0.35 to 0.65 molybdenum; no greater than 0.002 sulfur; no greater 65 than 0.015 phosphorus; no greater than 0.11 nitrogen; iron; and incidental impurities. In various embodiments, the steel alloys may also comprise 0.0002 to 0.0050 boron; 0.001 to 0.015 cerium; and/or 0.001 to 0.015 lanthanum.

In various embodiments, the carbon content may comprise any sub-range within 0.40 to 0.53 weight percent, such as, for example, 0.48 to 0.52 weight percent or 0.49 to 0.51 weight percent. The manganese content may comprise any sub-range within 0.15 to 1.00 weight percent, such as, for example, 0.20 to 0.80 weight percent. The silicon content may comprise any sub-range within 0.15 to 0.45 weight percent, such as, for example, 0.20 to 0.40 weight percent. The chromium content may comprise any sub-range within 0.95 to 1.70 weight percent, such as, for example, 1.00 to 1.50 weight percent. The nickel content may comprise any sub-range within 3.30 to 4.30 weight percent, such as, for example, 3.75 to 4.25 weight percent. The molybdenum content may comprise any sub-range within 0.35 to 0.65 weight percent, such as, for example, 0.40 to 0.60 weight percent.

In various embodiments, the sulfur content may comprise a content no greater than 0.001 weight percent, the phosphorus content may comprise a content no greater than 0.010 weight percent, and/or the nitrogen content may comprise a content no greater than 0.010 weight percent. In various embodiments, the boron content may comprise any sub-range within 0.0002 to 0.0050 weight percent, such as, for example, 0.008 to 0.0024, 0.0010 to 0.0030, or 0.0015 to 0.0025 weight percent. The cerium content may comprise any sub-range within 0.001 to 0.015 weight percent, such as, for example, 0.003 to 0.010 weight percent. The lanthanum content may comprise any sub-range within 0.001 to 0.015 weight percent, such as, for example, 0.002 to 0.010 weight percent.

In addition to developing a unique alloy system, the inventors also conducted studies, discussed below, to determine how one may process steels within the present disclosure to improve hardness and ballistic performance as evaluated per known military specifications MIL-DTL-46100E, MIL-A-46099C, and MIL-DTL-32332. The inventors also subjected samples of steel according to the present disclosure to various temperatures intended to dissolve carbide particles within the steel and to allow diffusion and produce an advantageous degree of homogeneity within the steel. An objective of this testing was to determine heat treating temperatures that do not produce excessive carburization or result in excessive and unacceptable grain growth, which would reduce material

transform the retained austenite to lower bainite and/or lath martensite. This may result in steel alloys having a synergistic combination of hard twinned martensite microstructure and tougher, more ductile lower bainite and/or lath martensite microstructure. A synergistic combination of hardness, toughness, and ductility may impart excellent ballistic penetration and crack resistance properties to the alloys described herein.

Trials evaluating the ballistic performance of samples cooled at different rates from austenitizing temperature, and therefore having differing hardnesses, also were conducted. The inventors' testing also included tempering trials and cooling trials intended to assess how best to promote multi-hit ballistic resistance with reduced, minimal, or zero crack propagation. Samples were evaluated by determining  $V_{50}$  ballistic limit values of the various test samples per MIL-DTL-46100E, MIL-A-46099C, and MIL-DTL-32332 using 7.62 mm (.30 caliber M2, AP) projectiles. Details of the inventors' alloy studies follow.

#### 1. Preparation of Experimental Alloy Plates

A novel composition for low-alloy steel armors was formulated. The present inventors concluded that such alloy composition preferably should include relatively high nickel content and low levels of sulfur, phosphorus, and nitrogen residual elements, and should be processed to plate form in a way that promotes homogeneity. Several ingots of an alloy having the experimental chemistry shown in Table 2 were prepared by argon-oxygen-decarburization ("AOD") or AOD and electroslag remelting ("ESR"). Table 2 indicates the desired minimum and maximum, a preferred minimum and a preferred maximum (if any), and a nominal aim level of the alloying elements, as well as the actual chemistry of the alloy produced. The balance of the alloy included iron and incidental impurities. Non-limiting examples of elements that may be present as incidental impurities include copper, aluminum, titanium, tungsten, and cobalt. Other potential incidental impurities, which may be derived from the starting materials and/or through alloy processing, will be known to persons having ordinary skill in metallurgy. Alloy compositions are reported in Table 2, and more generally are reported herein, as weight percentages based on total alloy weight unless otherwise indicated. Also, in Table 2, "LAP" refers to "low as possible".

TABLE 2

|           | C   | Mn   | P    | S     | Si  | Cr   | Ni   | Mo  | Ce   | La   | V   | W   | Ti   | Co  | Al   | N     | B     |
|-----------|-----|------|------|-------|-----|------|------|-----|------|------|-----|-----|------|-----|------|-------|-------|
| Min.      | .40 | .15  | —    | —     | .15 | .95  | 3.30 | .35 | .001 | .001 | —   | —   | —    | —   | —    | .0002 |       |
| Max.      | .53 | 1.00 | .015 | .002  | .45 | 1.70 | 4.30 | .65 | .015 | .015 | .05 | .08 | .05  | .05 | .020 | .010  | .0050 |
| Preferred | .49 | .20  | —    | —     | .20 | 1.00 | 3.75 | .40 | .003 | .002 | —   | —   | —    | —   | —    | —     | .0010 |
| Min.      |     |      |      |       |     |      |      |     |      |      |     |     |      |     |      |       |       |
| Preferred | .51 | .80  | .010 | .001  | .40 | 1.50 | 4.25 | .60 | .010 | .010 | —   | —   | —    | —   | —    | —     | .0030 |
| Max.      |     |      |      |       |     |      |      |     |      |      |     |     |      |     |      |       |       |
| Aim       | .50 | .50  | LAP  | LAP   | .30 | 1.25 | 4.00 | .50 | —    | —    | LAP | LAP | LAP  | LAP | LAP  | LAP   | .0016 |
| Actual*   | .50 | .53  | .01  | .0006 | 0.4 | 1.24 | 4.01 | .52 | —    | .003 | .01 | .01 | .002 | .02 | .02  | .007  | .0015 |

\*Analysis revealed that the composition also included 0.09 copper, 0.004 niobium, 0.004 tin, 0.001 zirconium, and 92.62 iron.

toughness and thereby degrade ballistic performance. In various processes, plates of the steel were cross rolled to provide some degree of isotropy.

It is also believed that various embodiments of the processing methods described herein impart a particular microstructure to the steel alloys. For example, in various embodiments, the disclosed steels are cooled from austenitizing temperatures to form martensite. The cooled alloys may contain a significant amount of twinned martensite and various amounts of retained austenite. Tempering of the cooled alloys according to various embodiments described herein may

ingot surfaces were ground using conventional practices. The ingots were then heated to about 1300° F. (704° C.), equalized, held at this first temperature for 6 to 8 hours, heated at about 200° F./hour (93° C./hour) up to about 2050° F. (1121° C.), and held at the second temperature for about 30-40 minutes per inch of thickness. Ingots were then hot rolled to 6-7 inches (15.2-17.8 cm) thickness, end cropped and, if necessary, reheated to about 2050° F. (1121° C.) for 1-2 hours before subsequent additional hot rolling to re-slabs of about 1.50-2.65 inches (3.81-6.73 cm) in thickness. The re-slabs were stress relief annealed using conventional prac-

## 11

ties, and slab surfaces were then blast cleaned and finish rolled to long plates having finished gauge thicknesses ranging from about 0.188 inches (4.8 mm) to about 0.310 inch (7.8 mm). The long plates were then fully annealed, blast cleaned, flattened, and sheared to form multiple individual plates.

In certain cases, the re-slabs were reheated to rolling temperature immediately before the final rolling step necessary to achieve finished gauge. More specifically, certain plate samples were final rolled as shown in Table 3. Tests were conducted on samples of the 0.275 and 0.310 inch (7 and 7.8 mm) gauge (nominal) plates that were final rolled as shown in Table 3 to assess possible heat treatment parameters optimizing surface hardness and ballistic performance properties.

TABLE 3

| Approx. Thickness, inch (mm) | Hot Rolling Process Parameters                                          |
|------------------------------|-------------------------------------------------------------------------|
| 0.275 (7)                    | Reheated slab at 0.5 for approx. 10 min. before rolling to finish gauge |
| 0.275 (7)                    | No re-heat immediately before rolling to finish gauge                   |
| 0.310 (7.8)                  | Reheated slab at 0.6 for approx. 30 min. before rolling to finish gauge |
| 0.310 (7.8)                  | No re-heat immediately before rolling to finish gauge                   |

## 2. Hardness Testing

Plates produced as in Section 1 above were subjected to an austenitizing treatment and a hardening step, cut into thirds to form samples for further testing and, optionally, subjected to a tempering treatment. The austenitizing treatment involved heating the samples to 1550-1650° F. (843-899° C.) for 40 minutes time-at-temperature. Hardening involved air-cooling the samples or quenching the samples in oil from the austenitizing treatment temperature to room temperature ("RT").

## 12

As used herein, the term "time-at-temperature" refers to the duration of the period of time that an article is maintained at a specified temperature after at least the surface of the article reaches that temperature. For example, the phrase "heating a sample to 1650° F. for 40 minutes time-at-temperature" means that the sample is heated to a temperature of 1650° F. and once the sample reaches 1650° F., the sample is maintained for 40 minutes at 1650°. After a specified time-at-temperature has elapsed, the temperature of an article may change from the specified temperature. As used herein, the term "minimum furnace time" refers to the minimum duration of the period of time that an article is located in a furnace that is heated to a specified temperature. For example, the phrase "heating a sample to 1650° F. for 40 minutes minimum furnace time" means that the sample is placed into a 1650° F. furnace for 40 minutes and then removed from the 1650° F. furnace.

One of the three samples from each austenitized and hardened plate was retained in the as-hardened state for testing. The remaining two samples cut from each austenitized and hardened plate were temper annealed by holding at either 250° F. (121° C.) or 300° F. (149° C.) for 90 minutes time-at-temperature. To reduce the time needed to evaluate sample hardness, all samples were initially tested using the Rockwell C (HR<sub>C</sub>) test rather than the Brinell hardness test. The two samples exhibiting the highest HR<sub>C</sub> values in the as-hardened state were also tested to determine Brinell hardness (BHN) in the as-hardened state (i.e., before any tempering treatment). Table 4 lists austenitizing treatment temperatures, quench type, gauge, and HR<sub>C</sub> values for samples tempered at either 250° F. (121° C.) or 300° F. (149° C.). Table 4 also indicates whether the plates used in the testing were subjected to reheating immediately prior to rolling to final gauge. In addition, Table 4 lists BHN hardness for the untempered, as-hardened samples exhibiting the highest HR<sub>C</sub> values in the as-hardened condition.

TABLE 4

| Aus. Anneal Temp. (°F.) | Cooling Type | Reheat | Gauge | As-Harden. HR <sub>C</sub> | As-Harden. BHN | HR <sub>C</sub> Post 250° F. Anneal | HR <sub>C</sub> Post 300° F. Anneal |
|-------------------------|--------------|--------|-------|----------------------------|----------------|-------------------------------------|-------------------------------------|
| 1550                    | Air          | No     | 0.275 | 50                         | —              | 54                                  | 54                                  |
| 1550                    | Air          | No     | 0.310 | 53                         | —              | 58                                  | 57                                  |
| 1550                    | Air          | Yes    | 0.275 | 50                         | —              | 53                                  | 56                                  |
| 1550                    | Air          | Yes    | 0.310 | 50                         | —              | 55                                  | 57                                  |
| 1550                    | Oil          | No     | 0.275 | 48                         | —              | 54                                  | 56                                  |
| 1550                    | Oil          | No     | 0.310 | 53                         | —              | 58                                  | 58                                  |
| 1550                    | Oil          | Yes    | 0.275 | 59                         | 624            | 52                                  | 53                                  |
| 1550                    | Oil          | Yes    | 0.310 | 59                         | —              | 55                                  | 58                                  |
| 1600                    | Air          | No     | 0.275 | 53                         | 587            | 54                                  | 57                                  |
| 1600                    | Air          | No     | 0.310 | 48                         | —              | 56                                  | 57                                  |
| 1600                    | Air          | Yes    | 0.275 | 54                         | —              | 56                                  | 57                                  |
| 1600                    | Air          | Yes    | 0.310 | 50                         | —              | 57                                  | 58                                  |
| 1600                    | Oil          | No     | 0.275 | 53                         | —              | 54                                  | 57                                  |
| 1600                    | Oil          | No     | 0.310 | 52                         | —              | 55                                  | 58                                  |
| 1600                    | Oil          | Yes    | 0.275 | 51                         | —              | 51                                  | 58                                  |
| 1600                    | Oil          | Yes    | 0.310 | 53                         | —              | 53                                  | 58                                  |
| 1650                    | Air          | No     | 0.275 | 46                         | —              | 54                                  | 56                                  |
| 1650                    | Air          | No     | 0.310 | 46                         | —              | 53                                  | 56                                  |
| 1650                    | Air          | Yes    | 0.275 | 48                         | —              | 53                                  | 57                                  |
| 1650                    | Air          | Yes    | 0.310 | 48                         | —              | 54                                  | 56                                  |
| 1650                    | Oil          | No     | 0.275 | 47                         | —              | 52                                  | 55                                  |
| 1650                    | Oil          | No     | 0.310 | 46                         | —              | 54                                  | 57                                  |
| 1650                    | Oil          | Yes    | 0.275 | 46                         | —              | 55                                  | 54                                  |
| 1650                    | Oil          | Yes    | 0.310 | 47                         | —              | 57                                  | 58                                  |

Table 5 provides average HRC values for the samples included in Table 4 in the as-hardened state and after temper anneals of either 250° F. (121° C.) or 300° F. (149° C.) for 90 minutes time-at-temperature.

TABLE 5

| Austenitizing Anneal Temp. (° F.) | Avg. HR <sub>c</sub> As-Hardened | Avg. HR <sub>c</sub> Post 250° F. Anneal | Avg. HR <sub>c</sub> Post 300° F. Anneal |
|-----------------------------------|----------------------------------|------------------------------------------|------------------------------------------|
| 1550                              | 52                               | 55                                       | 56                                       |
| 1600                              | 52                               | 55                                       | 57                                       |
| 1650                              | 47                               | 54                                       | 56                                       |

In general, Brinell hardness is determined per specification ASTM E-10 by forcing an indenter in the form of a hard steel or carbide sphere of a specified diameter under a specified load into the surface of the sample and measuring the diameter of the indentation left after the test. The Brinell hardness number or "BHN" is obtained by dividing the indenter load used (in kilograms) by the actual surface area of the indentation (in square millimeters). The result is a pressure measurement, but the units are rarely stated when BHN values are reported.

In assessing the Brinell hardness number of steel armor samples, a desk top machine is used to press a 10 mm diameter tungsten carbide sphere indenter into the surface of the test specimen. The machine applies a load of 3000 kilograms, usually for 10 seconds. After the ball is retracted, the diameter of the resulting round impression is determined. The BHN value is calculated according to the following formula:

$$\text{BHN} = \frac{2P}{\pi D(D - (D^2 - d^2)^{1/2})},$$

where BHN=Brinell hardness number; P=the imposed load in kilograms; D=the diameter of the spherical indenter in mm; and d=the diameter of the resulting indenter impression in millimeters.

Several BHN tests may be carried out on a surface region of an armor plate and each test might result in a slightly different hardness number. This variation in hardness can be due to minor variations in the local chemistry and microstructure of the plate since even homogenous armors are not absolutely uniform. Small variations in hardness measures also can result from errors in measuring the diameter of the indenter impression on the specimen. Given the expected variation of hardness measurements on any single specimen, BHN values often are provided as ranges, rather than as single discrete values.

As shown in Table 4, the highest Brinell hardnesses measured for the samples were 624 and 587. Those particular as-hardened samples were austenitized at 1550° F. (843° C.) (BHN 624) or 1600° F. (871° C.) (BHN 587). One of the two samples was oil quenched (BHN 624), and the other was air-cooled, and only one of the two samples (BHN 624) was reheated prior to rolling to final gauge.

In general, it was observed that using a temper anneal tended to increase sample hardness, with a 300° F. (149° C.) tempering temperature resulting in the greater hardness increase at each austenitizing temperature. Also, it was observed that increasing the austenitizing temperature generally tended to decrease the final hardness achieved. These correlations are illustrated in FIG. 1, which plots average HR<sub>c</sub> hardness as a function of austenitizing temperature for 0.275 inch (7 mm) samples (left panel) and 0.310 inch (7.8 mm) samples (right panel) in the as-hardened state ("AgeN") or after tempering at either 250° F. (121° C.) ("Age25") or 300° F. (149° C.) ("Age30").

FIGS. 2 and 3 consider the effects on hardness of quench type and whether the re-slabs were reheated prior to rolling to 0.275 and 0.310 inch (7 and 7.8 mm) nominal final gauge. FIG. 2 plots HR<sub>c</sub> hardness as a function of austenitizing temperature for non-reheated 0.275 inch (7 mm) samples (upper left panel), reheated 0.275 inch (7 mm) samples (lower left panel), non-reheated 0.310 inch (7.8 mm) samples (upper right panel), and reheated 0.310 inch (7.8 mm) samples (lower right panel) in the as-hardened state ("AgeN") or after tempering at either 250° F. (121° C.) ("Age25") or 300° F. (149° C.) ("Age30"). Similarly, FIG. 3 plots HR<sub>c</sub> hardness as a function of austenitizing temperature for air-cooled 0.275 inch (7 mm) samples (upper left panel), oil-quenched 0.275 inch (7 mm) samples (lower left panel), air-cooled 0.310 inch (7.8 mm) samples (upper right panel), and oil-quenched 0.310 inch (7.8 mm) samples (lower right panel) in the as-hardened state ("AgeN") or after tempering at either 250° F. (121° C.) ("Age25") or 300° F. (149° C.) ("Age30"). The average hardness of samples processed at each of the austenitizing temperatures and satisfying the conditions pertinent to each of the panels in FIGS. 2 and 3 is plotted in each panel as a square-shaped data point, and each such data point in each panel is connected by dotted lines so as to better visualize any trend. The overall average hardness of all samples considered in each panel of FIGS. 2 and 3 is plotted in each panel as a diamond-shaped data point.

With reference to FIG. 2, it was generally observed that the hardness effect of reheating prior to rolling to final gauge was minor and not evident relative to the effect of other variables. For example, only one of the samples with the highest two Brinell hardnesses had been reheated prior to rolling to final gauge. With reference to FIG. 3, it was generally observed that any hardness difference resulting from using an air cool versus an oil quench after the austenitizing heat treatment was minimal. For example, only one of the samples with the highest two Brinell hardnesses had been reheated in plate form prior to rolling to final gauge.

It was determined that the experimental alloy samples included a high concentration of retained austenite after the austenitizing anneals. Greater plate thickness and higher austenitizing treatment temperatures tended to produce greater retained austenite levels. Also, it was observed that at least some portion of the austenite transformed to martensite during the temper annealing. Any untempered martensite present after the temper annealing treatment may lower the toughness of the final material. To better ensure optimum toughness, it was concluded that an additional temper anneal could be used to further convert any retained austenite to martensite. Based on the inventors' observations, an austenitizing temperature of at least about 1500° F. (815° C.), and more preferably at least about 1550° F. (843° C.), appears to be satisfactory for the articles evaluated in terms of achieving high hardnesses.

**3. Ballistic Performance Testing**  
Several 18×18 inch (45.7×45.7 cm) test panels having a nominal thickness of 0.275 inch (7 mm) were prepared as described in Section 1 above, and then further processed as discussed below. The panels were then subjected to ballistic performance testing as described below.

Eight test panels produced as described in Section 1 were further processed as follows. The eight panels were austenitized at 1600° F. (871° C.) for 35 minutes (+/- 5 minutes), allowed to air cool to room temperature, and hardness tested. The BHN hardness of one of the eight panels austenitized at 1600° F. (871° C.) was determined after air cooling in the as-austenitized, un-tempered ("as-hardened") condition. The as-hardened panel exhibited a hardness of about 600 BHN.

Six of the eight panels austenitized at 1600° F. (871° C.) and air cooled were divided into three sets of two, and each set was tempered at one of 250° F. (121° C.), 300° F. (149° C.), and 350° F. (177° C.) for 90 minutes (+/-5 minutes), air cooled to room temperature, and hardness tested. One panel of each of the three sets of tempered panels (three panels total) was set aside, and the remaining three tempered panels were re-tempered at their original 250° F. (121° C.), 300° F. (149° C.), or 350° F. (177° C.) tempering temperature for 90 minutes (+/-5 minutes), air cooled to room temperature, and hardness tested. These six panels are identified in Table 6 below by samples ID numbers 1 through 6.

One of the eight panels austenitized at 1600° F. (871° C.) and air cooled was immersed in 32° F. (0° C.) ice water for approximately 15 minutes and then removed and hardness tested. The panel was then tempered at 300° F. (149° C.) for 90 minutes (+/-5 minutes), air cooled to room temperature, immersed in 32° F. (0° C.) ice water for approximately 15 minutes, and then removed and hardness tested. The sample was then re-tempered at 300° F. (149° C.) for 90 minutes (+/-5 minutes), air cooled to room temperature, again placed in 32° F. (0° C.) ice water for approximately 15 minutes, and then again removed and hardness tested. This panel is referenced in Table 6 by ID number 7.

Three additional test panels prepared as described in Section 1 above were further processed as follows and then subjected to ballistic performance testing. Each of the three panels was austenitized at 1950° F. (1065° C.) for 35 minutes (+/-5 minutes), allowed to air cool to room temperature, and hardness tested. Each of the three panels was next tempered at 300° F. for 90 minutes (+/-5 minutes), air cooled to room temperature, and hardness tested. Two of three tempered, air-cooled panels were then re-tempered at 300° F. (149° C.) for 90 minutes (+/-5 minutes), air cooled, and then tested for hardness. One of the re-tempered panels was next cryogenically cooled to -120° F. (-84° C.), allowed to warm to room temperature, and hardness tested. These three panels are identified by ID numbers 9-11 in Table 6.

The eleven panels identified in Table 6 were individually evaluated for ballistic performance by assessing  $V_{50}$  ballistic limit (protection) using 7.62 mm (.30 caliber M2, AP) projectiles as per MIL-DTL-46100E. The  $V_{50}$  ballistic limit value is the calculated projectile velocity at which the probability is 50% that the projectile will penetrate the armor test panel.

More precisely, under U.S. Military Specifications MIL-DTL-46100E ("Armor, Plate, Steel, Wrought, High Hardness"), MIL-A-46099C ("Armor Plate, Steel, Roll-Bonded, Dual Hardness (0.187 Inches To 0.700 Inches Inclusive")), and MIL-DTL-32332 ("Armor Plate, Steel, Wrought, Ultra-

high-hardness"), the  $V_{50}$  ballistic limit (protection) value is the average velocity of six fair impact velocities comprising the three lowest projectile velocities resulting in complete penetration and the three highest projectile velocities resulting in partial penetration. A maximum spread of 150 feet-per-second (fps) is permitted between the lowest and highest velocities employed in determining  $V_{50}$  ballistic limit values.

In cases where the lowest complete penetration velocity is lower than the highest partial penetration velocity by more than 150 fps, the ballistic limit is based on ten velocities (the five lowest velocities that result in complete penetration and the five highest velocities that result in partial penetrations). When the ten-round excessive spread ballistic limit is used, the velocity spread must be reduced to the lowest partial level, and as close to 150 fps as possible. The normal up and down firing method is used in determining  $V_{50}$  ballistic limit (protection) values, all velocities being corrected to striking velocity. If the computed  $V_{50}$  ballistic limit value is less than 30 fps above the minimum required and if a gap (high partial penetration velocity below the low complete penetration velocity) of 30 fps or more exists, projectile firing is continued as needed to reduce the gap to 25 fps or less.

The  $V_{50}$  ballistic limit value determined for a test panel may be compared with the required minimum  $V_{50}$  ballistic limit value for the particular thickness of the test panel. If the calculated  $V_{50}$  ballistic limit value for the test panel exceeds the required minimum  $V_{50}$  ballistic limit value, then it may be said that the test panel has "passed" the requisite ballistic performance criteria. Minimum  $V_{50}$  ballistic limit values for plate armor are set out in various U.S. military specifications, including MIL-DTL-46100E, MIL-A-46099C, and MIL-DTL-32332.

Table 6 lists the following information for each of the eleven ballistic test panels: sample ID number; austenitizing temperature; BHN hardness after cooling to room temperature from the austenitizing treatment ("as-hardened"); tempering treatment parameters (if used); BHN hardness after cooling to room temperature from the tempering temperature; re-tempering treatment parameters (if used); BHN hardness after cooling to room temperature from the re-tempering temperature; and the difference in fps between the panel's calculated  $V_{50}$  ballistic limit value and the required minimum  $V_{50}$  ballistic limit value as per MIL-DTL-46100E and as per MIL-A-46099C. Positive  $V_{50}$  difference values in Table 6 (e.g., "+419") indicate that the calculated  $V_{50}$  ballistic limit for a panel exceeded the required  $V_{50}$  by the indicated extent. Negative difference values (e.g., "-44") indicate that the calculated  $V_{50}$  ballistic limit value for the panel was less than the required  $V_{50}$  ballistic limit value per the indicated military specification by the indicated extent.

TABLE 6

| ID | Aus. Temp. (°F.) | As-Hardened Hardness (BHN) | Temper (minutes @ ° F.) | Post-Temper Hardness (BHN) |                         | Post Re-Temper Hardness (BHN) |                         | Post Re-Temper Hardness (BHN) | V <sub>50</sub> versus 46100E (fps) | V <sub>50</sub> versus 46099C (fps) |
|----|------------------|----------------------------|-------------------------|----------------------------|-------------------------|-------------------------------|-------------------------|-------------------------------|-------------------------------------|-------------------------------------|
|    |                  |                            |                         | Temper (minutes @ ° F.)    | Temper (minutes @ ° F.) | Temper (minutes @ ° F.)       | Temper (minutes @ ° F.) |                               |                                     |                                     |
| 1  | 1600             | 600                        | 90 @ 250                | 600                        | NA                      | NA                            | NA                      | NA                            | +419                                | +37                                 |
| 2  | 1600             | 600                        | 90 @ 250                | 600                        | 90 @ 250                | 600                           | NA                      | NA                            | +341                                | -44                                 |
| 3  | 1600             | 600                        | 90 @ 300                | 600                        | NA                      | NA                            | NA                      | NA                            | +309                                | +74                                 |
| 4  | 1600             | 600                        | 90 @ 300                | 600                        | 90 @ 300                | 600                           | NA                      | NA                            | +346                                | -38                                 |
| 5  | 1600             | 600                        | 90 @ 350                | 578                        | NA                      | NA                            | NA                      | NA                            | +231                                | -153                                |
| 6  | 1600             | 600                        | 90 @ 350                | 578                        | 90 @ 350                | 578                           | NA                      | NA                            | +240                                | -144                                |
| 7  | 1600             | 600                        | 15 @ 32                 | 600                        | 90 @ 300                | 600                           | 90 @ 300                | 600                           | +372                                | -16                                 |
|    |                  |                            |                         |                            | +AC +                   | +AC +                         | +AC +                   |                               |                                     |                                     |
|    |                  |                            |                         |                            | 15 @ 32                 | 15 @ 32                       | 15 @ 32                 |                               |                                     |                                     |
| 8  | 1950             | 555                        | 90 @ 300                | 555                        | NA                      | NA                            | NA                      | NA                            | +243                                | -137                                |

TABLE 6-continued

| ID | Aus. Temp. (°F.) | As-Hardened            |                | Post-Temper            |                | Post Re-Temper         |                | Post Re-Temper Hardness (BHN) | V <sub>50</sub> versus 46100E (fps) | V <sub>50</sub> versus 46099C (fps) |
|----|------------------|------------------------|----------------|------------------------|----------------|------------------------|----------------|-------------------------------|-------------------------------------|-------------------------------------|
|    |                  | Temper (minutes @ °F.) | Hardness (BHN) | Temper (minutes @ °F.) | Hardness (BHN) | Temper (minutes @ °F.) | Hardness (BHN) |                               |                                     |                                     |
| 9  | 1950             | 555                    | 90 @ 300       | 555                    | 90 @ 300       | 555                    | NA             | NA                            | +234                                | -147                                |
| 10 | 1950             | 555                    | 90 @ 300       | —                      | 90 @ 300       | —                      | -120           | —                             | —                                   | —                                   |

Eight additional 18×18 inch (45.7×45.7 cm) (nominal) test panels, numbered 12-19, composed of the experimental alloy were prepared as described in Section 1 above. Each of the panels was nominally either 0.275 inch (7 mm) or 0.320 inch (7.8 mm) in thickness. Each of the eight panels was subjected to an austenitizing treatment by heating at 1600° F. (871° C.) for 35 minutes (+/-5 minutes) and then air cooled to room temperature. Panel 12 was evaluated for ballistic performance in the as-hardened state (as-cooled, with no temper treatment) against 7.62 mm (.30 caliber) M2, AP projectiles. Panels 13-19 were subjected to the individual tempering steps listed in Table 7, air cooled to room temperature, and then evaluated for ballistic performance in the same way as panels 1-11 above. Each of the tempering times listed in Table 7 are approximations and were actually within +/-5 minutes of the listed durations. Table 8 lists the calculated V<sub>50</sub> ballistic limit (performance) values of each of test panels 12-19, along with the required minimum V<sub>50</sub> ballistic limit value as per MIL-DTL-46100E and as per MIL-A-46099C for the particular panel thickness listed in Table 7.

no greater than  $\frac{3}{16}$  inch and a width of at least 10 inches. Persons having ordinary skill will readily understand the differences between the various conventional mill products, such as plate, sheet, and bar.

#### 4. Cooling Tests

##### a. Trial 1

Groups of 0.275×18×18 inch samples having the actual chemistry shown in Table 2 were processed through an austenitizing cycle by heating the samples at 1600±10° F. (871±6° C.) for 35 minutes±5 minutes, and were then cooled to room temperature using different methods to influence the cooling path. The cooled samples were then tempered for a defined time, and allowed to air cool to room temperature. The samples were Brinell hardness tested and ballistic tested. Ballistic V<sub>50</sub> values meeting the requirements under specification MIL-DTL-46100E were desired. Preferably, the ballistic performance as evaluated by ballistic V<sub>50</sub> values is no less 150 fps less than the V<sub>50</sub> values required under specification MIL-A-46099C. In general, MIL-A-46099C requires significantly higher V<sub>50</sub> values that are generally 300-400 fps greater than required under MIL-DTL-46100E.

TABLE 7

| ID | Gauge (inch) | No Temper | Temper @ 175° F. for 60 minutes | Temper @ 200° F. for 60 minutes | Temper @ 225° F. for 60 minutes | Temper @ 250° F. for 30 minutes | Temper @ 250° F. for 60 minutes | Temper @ 250° F. for 90 minutes | Temper @ 250° F. for 120 minutes |
|----|--------------|-----------|---------------------------------|---------------------------------|---------------------------------|---------------------------------|---------------------------------|---------------------------------|----------------------------------|
|    |              |           |                                 |                                 |                                 |                                 |                                 |                                 |                                  |
| 12 | 0.282        | X         |                                 |                                 |                                 |                                 |                                 |                                 |                                  |
| 13 | 0.280        |           | X                               |                                 |                                 |                                 |                                 |                                 |                                  |
| 14 | 0.281        |           |                                 | X                               |                                 |                                 |                                 |                                 |                                  |
| 15 | 0.282        |           |                                 |                                 | X                               |                                 |                                 |                                 |                                  |
| 16 | 0.278        |           |                                 |                                 |                                 | X                               |                                 |                                 |                                  |
| 17 | 0.278        |           |                                 |                                 |                                 |                                 | X                               |                                 |                                  |
| 18 | 0.285        |           |                                 |                                 |                                 |                                 |                                 | X                               |                                  |
| 19 | 0.281        |           |                                 |                                 |                                 |                                 |                                 |                                 | X                                |

TABLE 8

| Sample ID | Calculated V <sub>50</sub> Ballistic Limit (fps) | Min. V <sub>50</sub> Ballistic Limit per | Min. V <sub>50</sub> Ballistic Limit per |
|-----------|--------------------------------------------------|------------------------------------------|------------------------------------------|
|           |                                                  | MIL-DTL-46100E (fps)                     | MIL-A-46099C (fps)                       |
| 12        | 2936                                             | 2426                                     | 2807                                     |
| 13        | 2978                                             | 2415                                     | 2796                                     |
| 14        | 3031                                             | 2421                                     | 2801                                     |
| 15        | 2969                                             | 2426                                     | 2807                                     |
| 16        | 2877                                             | 2403                                     | 2785                                     |
| 17        | 2915                                             | 2403                                     | 2785                                     |
| 18        | 2914                                             | 2443                                     | 2823                                     |
| 19        | 2918                                             | 2421                                     | 2801                                     |

Mill products in the forms of, for example, plate, bars, and sheet may be made from the alloys according to the present disclosure by processing including steps formulated with the foregoing observations and conclusions in mind in order to optimize hardness and ballistic performance of the alloy. As is understood by those having ordinary skill, a "plate" product has a nominal thickness of at least  $\frac{3}{16}$  inch and a width of at least 10 inches, and a "sheet" product has a nominal thickness

no greater than  $\frac{3}{16}$  inch and a width of at least 10 inches. Persons having ordinary skill will readily understand the differences between the various conventional mill products, such as plate, sheet, and bar.

Table 9 lists hardness and V<sub>50</sub> results for samples cooled from the austenitizing temperature by vertically racking the samples on a cooling rack with 1 inch spacing between the samples and allowing the samples to cool to room temperature in still air in a room temperature environment. FIG. 4 schematically illustrates the stacking arrangement for these samples.

Table 10 provides hardness and V<sub>50</sub> values for samples cooled from the austenitizing temperature using the same general cooling conditions and the same vertical samples racking arrangement of the samples in Table 9, but wherein a cooling fan circulated room temperature air around the samples. Thus, the average rate at which the samples listed in Table 10 cooled from the austenitizing temperature exceeded that of the samples listed in Table 9.

Table 11 lists hardnesses and V<sub>50</sub> results for still air-cooled samples arranged horizontally on the cooling rack and stacked in contact with adjacent samples so as to influence the rate at which the samples cooled from the austenitizing temperature. The V<sub>50</sub> values included in Table 11 are plotted as a function of tempering practice in FIG. 6. Four different stack-

ing arrangements were used for the samples of Table 11. In one arrangement, shown on the top portion of FIG. 5, two samples were placed in contact with one another. In another arrangement, shown in the bottom portion of FIG. 5, three samples were placed in contact with one another. FIG. 8 is a plot of the cooling curves for the samples stacked as shown in the top and bottom portions of FIG. 5. FIG. 7 shows two additional stacking arrangements wherein either four plates (top portion) or five plates (bottom portion) were placed in contact with one another while cooling from the austenitizing temperature. FIG. 9 is a plot of the cooling curves for the samples stacked as shown in the top and bottom portions of FIG. 7.

For each sample listed in Table 11, the second column of the table indicates the total number of samples associated in the stacking arrangement. It is expected that circulating air around the samples (versus cooling in still air) and placing differing numbers of samples in contact with one another, as with the samples in Tables 9, 10, and 11, influenced the shape of the cooling curves for the various samples. In other words, it is expected that the particular paths followed by the cooling curves (i.e., the "shapes" of the curves) differed for the various arrangements of samples in Tables 9, 10, and 11. For example, the cooling rate in one or more regions of the cooling curve for a sample cooled in contact with other samples may be less than the cooling rate for a vertically racked, spaced-apart sample in the same cooling curve region. It is believed that the differences in cooling of the samples resulted in microstructural differences in the samples that unexpectedly influenced the ballistic penetration resistance of the samples, as discussed below.

Tables 9-11 identify the tempering treatment used with each sample listed in those tables. The  $V_{50}$  results in Tables 9-11 are listed as a difference in feet/second (fps) relative to the required minimum  $V_{50}$  ballistic limit value for the particular test sample size under specification MIL-A-46099C. As examples, a value of "-156" means that the  $V_{50}$  ballistic limit value for the sample, evaluated per the military specification using 7.62 mm (.30 caliber M2, AP) ammunition, was 156 fps less than the required value under the military specification, and a value of "+82" means that the  $V_{50}$  ballistic limit value exceeded the required value by 82 fps. Thus, large, positive difference values are most desirable as they reflect ballistic penetration resistance that exceeds the required  $V_{50}$  ballistic limit value under the military specification. The  $V_{50}$  values reported in Table 9 were estimated since the target plates cracked (degraded) during the ballistic testing. Ballistic results of samples listed in Tables 9 and 10 experienced a higher incidence of cracking.

TABLE 9

| Still Air Cooled, Samples Racked Vertically with 1 Inch Spacing |                                                   |                |                                      |                                     |
|-----------------------------------------------------------------|---------------------------------------------------|----------------|--------------------------------------|-------------------------------------|
| Sample                                                          | Temper Treatment (° F. temp/time-at-temp/cooling) | $V_{50}$ (fps) | Average Hardness (BHN) after Austen. | Average Hardness (BHN) after Temper |
| 79804AB1                                                        | 200/60/AC                                         | —              | 712                                  | 712                                 |
| 79804AB2                                                        | 200/60/AC +                                       | —              | 712                                  | 712                                 |
|                                                                 | 350/60/AC                                         | +3             | 712                                  | 640                                 |
| 79804AB3                                                        | 200/60/AC                                         | —              | 712                                  | 704                                 |
| 79804AB4                                                        | 200/60/AC                                         | —              | 712                                  | 712                                 |
| 79804AB5                                                        | 225/60/AC                                         | —              | 712                                  | 712                                 |
| 79804AB6                                                        | 225/60/AC                                         | —              | 712                                  | 704                                 |
| 79804AB7                                                        | 225/60/AC                                         | —              | 712                                  | 712                                 |
| 79804AB8                                                        | 400/60/AC                                         | -155           | 712                                  | 608                                 |
| 79804AB9                                                        | 500/60/AC                                         | -61            | 712                                  | 601                                 |
| 79804AB10                                                       | 600/60/AC                                         | -142           | 712                                  | 601                                 |

TABLE 10

| Fan Cooled, Samples Racked Vertically with 1 Inch Spacing |                                                   |                            |                                      |                                     |
|-----------------------------------------------------------|---------------------------------------------------|----------------------------|--------------------------------------|-------------------------------------|
| Sample                                                    | Temper Treatment (° F. temp/time-at-temp/cooling) | $V_{50}$ (estimated) (fps) | Average Hardness (BHN) after Austen. | Average Hardness (BHN) after Temper |
| 79373AB1                                                  | 200/60/AC                                         | -95                        | 712                                  | 675                                 |
| 79373AB2                                                  | 200/120/AC                                        | -47                        | 712                                  | 675                                 |
| 79373AB3                                                  | 225/60/AC                                         | +35                        | 712                                  | 668                                 |
| 79373AB4                                                  | 225/120/AC                                        | -227                       | 712                                  | 682                                 |
| 79373AB5                                                  | 250/60/AC                                         | +82                        | 712                                  | 682                                 |
| 79373AB6                                                  | 250/120/AC                                        | +39                        | 712                                  | 682                                 |
| 79373AB7                                                  | 275/60/AC                                         | +82                        | 712                                  | 682                                 |
| 79373AB8                                                  | 275/120/AC                                        | +13                        | 712                                  | 675                                 |
| 79373AB9                                                  | 300/60/AC                                         | -54                        | 712                                  | 675                                 |

TABLE 11

| Still Air Cooled, Stacked Samples |                                 |                                                   |                         |                                                                          |
|-----------------------------------|---------------------------------|---------------------------------------------------|-------------------------|--------------------------------------------------------------------------|
| Sample                            | Stacking (no. of sample plates) | Temper Treatment (° F. temp/time-at-temp/cooling) | $V_{50}$ (46099C) (fps) | Average Hardness (BHN) after Austen. Average Hardness (BHN) after Temper |
| 79804AB3                          | 2                               | 225/60/AC                                         | +191                    | 653 653                                                                  |
| 79804AB4                          | 2                               | 225/60/AC                                         | +135                    | 653 653                                                                  |
| 79804A81                          | 3                               | 225/60/AC                                         | +222                    | 640 627                                                                  |
| 79804AB5                          | 3                               | 225/60/AC                                         | +198                    | 640 640                                                                  |
| 79804AB6                          | 3                               | 225/60/AC                                         | +167                    | 627 627                                                                  |
| 79804AB7                          | 4                               | 225/60/AC                                         | +88                     | 646 646                                                                  |
| 79373DA1                          | 4                               | 225/60/AC                                         | +97                     | 601 601                                                                  |
| 79373DA2                          | 4                               | 225/60/AC                                         | -24                     | 601 601                                                                  |
| 79373DA3                          | 4                               | 225/60/AC                                         | +108                    | 620 607                                                                  |
| 79373DA4                          | 5                               | 225/60/AC                                         | +114                    | 627 614                                                                  |
| 79373DA5                          | 5                               | 225/60/AC                                         | +133                    | 627 601                                                                  |

TABLE 11-continued

| Still Air Cooled, Stacked Samples |                                          |                                                             |                                      |                                               |                                              |
|-----------------------------------|------------------------------------------|-------------------------------------------------------------|--------------------------------------|-----------------------------------------------|----------------------------------------------|
| Sample                            | Stacking<br>(no. of<br>sample<br>plates) | Temper<br>Treatment (° F.<br>temp/time-at-<br>temp/cooling) | V <sub>50</sub><br>(46099C)<br>(fps) | Average<br>Hardness<br>after Austen.<br>(BHN) | Average<br>Hardness<br>after Temper<br>(BHN) |
| 79373DA6                          | 5                                        | 225/60/AC                                                   | +138                                 | 620                                           | 601                                          |
| 79373DA7                          | 5                                        | 225/60/AC                                                   | +140                                 | 620                                           | 614                                          |
| 79373DA8                          | 5                                        | 225/60/AC                                                   | +145                                 | 614                                           | 621                                          |

Hardness values for the samples listed in Table 11 were significantly less than those for the samples of Tables 9 and 10. This difference was believed to be a result of placing samples in contact with one another when cooling the samples from the austenitizing temperature, which modified the cooling curve of the samples relative to the "air quenched" samples referenced in Tables 9 and 10 and FIG. 4. The slower cooling used for samples in Table 11 is also thought to act to auto-temper the material during the cooling from the austenitizing temperature to room temperature.

As discussed above, the conventional belief is that increasing the hardness of a steel armor enhances the ability of the armor to fracture impacting projectiles, and thereby should improve ballistic performance as evaluated, for example, by V<sub>50</sub> ballistic limit value testing. The samples in Tables 9 and 10 were compositionally identical to those in Table 11 and, with the exception of the manner of cooling from the austenitizing temperature, were processed in substantially the same manner. Therefore, persons having ordinary skill in the production of steel armor materials would expect that the reduced surface hardness of the samples in Table 11 would negatively impact ballistic penetration resistance and result in lower V<sub>50</sub> ballistic limit values relative to the samples in Tables 9 and 10.

Instead, the present inventors found that the samples of Table 11 unexpectedly demonstrated significantly improved penetration resistance, with a lower incidence of cracking while maintaining positive V<sub>50</sub> values. Considering the apparent improvement in ballistic properties in the experimental trials when tempering the steel after cooling from the austenitizing temperature, it is believed that in various embodiments of mill-scale runs it would be beneficial to temper at 250-450° F., and preferably at about 375° F., for about 1 hour after cooling from the austenitizing temperature.

The average V<sub>50</sub> ballistic limit value in Table 11 is 119.6 fps greater than the required V<sub>50</sub> ballistic limit value for the samples under MIL-A-46099C. Accordingly, the experimental data in Table 11 shows that embodiments of steel armors according to the present disclosure have V<sub>50</sub> velocities that approach or exceed the required values under MIL-A-46099C. In contrast, the average V<sub>50</sub> ballistic limit value listed in Table 10 for the samples cooled at a higher rate was only 2 fps greater than that required under the specification, and the samples experienced unacceptable multi-hit crack resistance. Given that the V<sub>50</sub> ballistic limit value requirements of MIL-A-46099C are approximately 300-400 fps greater than under specification MIL-DTL-46100E, various steel armor embodiments according to the present disclosure will also approach or meet the required values under MIL-DTL-46100E. Although in no way limiting to the invention in the present disclosure, the V<sub>50</sub> ballistic limit values preferably are no less than 150 fps less than the required values under MIL-A-46099C. In other words, the V<sub>50</sub> ballistic limit values preferably are at least as great as a V<sub>50</sub> value 150 fps less than

the required V<sub>50</sub> value under specification MIL-A-46099C with minimal crack propagation

The average penetration resistance performance of the embodiments of Table 11 is substantial and is believed to be at least comparable to certain more costly high alloy armor materials, or K-12®dual hardness armor plate. In sum, although the steel armor samples in Table 11 had significantly lower surface hardness than the samples in Tables 9 and 10, they unexpectedly demonstrated substantially greater ballistic penetration resistance, with reduced incidence to crack propagation, which is comparable to ballistic resistance of certain premium, high alloy armor alloys.

Without intending to be bound by any particular theory, the inventors believe that the unique composition of the steel armors according to the present disclosure and the non-conventional approach to cooling the armors from the austenitizing temperature are important to providing the steel armors with unexpectedly high penetration resistance. The inventors observed that the substantial ballistic performance of the samples in Table 11 was not merely a function of the samples' lower hardness relative to the samples in Tables 9 and 10. In fact, as shown in Table 12 below, certain of the samples in Table 9 had post-temper hardness that was substantially the same as the post-temper hardness of samples in Table 11, but the samples in Table 11, which were cooled from austenitizing temperature differently than the samples in Tables 9 and 10, had substantially higher V<sub>50</sub> ballistic limit values with lower incidence of cracking. Therefore, without intending to be bound by any particular theory of operation, it is believed that the significant improvement in penetration resistance in Table 11 may have resulted from an unexpected and significant microstructural change that occurred during the unconventional manner of cooling and additionally permitted the material to become auto-tempered while cooling to room temperature.

Although in the present trials the cooling curve was modified from that of a conventional air quench step by placing the samples in contact with one another in a horizontal orientation on the cooling rack, based on the inventors' observations discussed herein it is believed that other means of modifying the conventional cooling curve may be used to beneficially influence the ballistic performance of the alloys according to the present disclosure. Examples of possible ways to beneficially modify the cooling curve of the alloys include cooling from the austenitizing temperature in a controlled cooling zone or covering the alloy with a thermally insulating material such as, for example, Kaowool material, during all or a portion of the step of cooling the alloy from the austenitizing temperature.

TABLE 12

| Table 9 - Selected Samples       |                                 | Table 11 - Selected Samples      |                                 |
|----------------------------------|---------------------------------|----------------------------------|---------------------------------|
| Avg. Hardness after Temper (BHN) | V <sub>50</sub> (460/99C) (fps) | Avg. Hardness after Temper (BHN) | V <sub>50</sub> (460/99C) (fps) |
| 640                              | +3                              | 640                              | +198                            |
| 608                              | -155                            | 607                              | +108                            |
| 601                              | -61                             | 601                              | +97                             |
| 601                              | -142                            | 601                              | -24                             |
|                                  |                                 | 601                              | +133                            |
|                                  |                                 | 601                              | +138                            |

In light of advantages obtained by high hardness in armor applications, low alloy steels according to the present disclosure may have hardness of at least 550 BHN, and in various embodiments at least 570 BHN or 600 BHN. Based on the foregoing test results and the present inventors' observation,

sample (DA-8) of the racked samples. A second thermocouple (channel 2) was positioned on the outside face (i.e., not facing the middle plate) of an outer plate (DA-7). In a second arrangement, shown in FIG. 11, three samples were horizontally stacked in contact with one another, with sample no. DA-10 on the bottom, sample no. BA-2 on the top, and sample no. BA-1 in the middle. A first thermocouple (channel 3) was disposed on the top surface of the bottom sample, and a second thermocouple (channel 4) was disposed on the bottom surface of the top sample (opposite the top surface of the middle sample). After each arrangement of samples was heated to and held at the austenitizing temperature, the sample tray was removed from the furnace and allowed to cool in still air until the samples were below 300° F. (149° C.).

Hardness (BHN) was evaluated at corner locations of each sample after cooling the samples from the austenitizing temperature to room temperature, and again after each austenitized sample was tempered for 60 minutes at 225° F. (107° C.). Results are shown in Table 13.

TABLE 13

| Samples                     | Hardness (BHN) at Sample Corners after Cooling from Austenitizing Temperature |     |     |     | Hardness (BHN) at Sample Corners after Tempering Treatment |     |     |     |
|-----------------------------|-------------------------------------------------------------------------------|-----|-----|-----|------------------------------------------------------------|-----|-----|-----|
| <u>Vertically Stacked</u>   |                                                                               |     |     |     |                                                            |     |     |     |
| DA-7                        | 653                                                                           | 601 | 653 | 653 | 653                                                        | 627 | 601 | 627 |
| DA-8                        | 627                                                                           | 601 | 653 | 627 | 653                                                        | 627 | 653 | 653 |
| DA-9                        | 653                                                                           | 653 | 653 | 627 | 601                                                        | 627 | 601 | 627 |
| <u>Horizontally Stacked</u> |                                                                               |     |     |     |                                                            |     |     |     |
| DA-10 (bottom)              | 653                                                                           | 653 | 627 | 627 | 653                                                        | 627 | 601 | 653 |
| BA-1 (middle)               | 653                                                                           | 653 | 653 | 653 | 682                                                        | 682 | 653 | 653 |
| BA-2 (top)                  | 712                                                                           | 653 | 653 | 653 | 653                                                        | 653 | 653 | 653 |

steels according to the present invention may have hardness that is greater than 550 BHN and less than 700 BHN, and in various embodiments is greater than 550 or 570 BHN and less than 675. According to various other embodiments, steels according to the present disclosure have hardness that is at least 600 BHN and is less than 675 BHN. Hardness likely plays an important role in establishing ballistic performance. However, the experimental armor alloys produced according to the present methods also derive their unexpected substantial penetration resistance from microstructural changes resulting from the unconventional manner of cooling the samples, which modified the samples' cooling curves from a curve characterizing a conventional step of cooling samples from austenitizing temperature in air.

#### b. Trial 2

An experimental trial was conducted to investigate specific changes to the cooling curves of alloys cooled from the austenitizing temperature that may be at least partially responsible for the unexpected improvement in ballistic penetration resistance of alloys according to the present disclosure. Two groups of three 0.310 inch sample plates having the actual chemistry shown in Table 2 were heated to a 1600±10° F. (871±6° C.) austenitizing temperature for 35 minutes±5 minutes. The groups were organized on the furnace tray in two different arrangements to influence the cooling curve of the samples from the austenitizing temperature. In a first arrangement illustrated in FIG. 10, three samples (nos. DA-7, DA-8, and DA-9) were vertically racked with a minimum of 1 inch spacing between the samples. A first thermocouple (referred to as "channel 1") was positioned on the face of the middle

40 The cooling curve shown in FIG. 12 plots sample temperature recorded at each of channels 1-4 from a time just after the samples were removed from the austenitizing furnace until reaching a temperature in the range of about 200-400° F. (93-204° C.). FIG. 12 also shows a possible continuous cooling transformation (CCT) curve for the alloy, illustrating various phase regions for the alloy as it cools from high temperature. FIG. 13 shows a detailed view of a portion of the cooling curve of FIG. 11 including the region in which each of the cooling curves for channels 1-4 intersect the theoretical CCT curve. Likewise, FIG. 14 shows a portion of the cooling curve and CCT curves shown in FIG. 12, in the 500-900° F. (260-482° C.) sample temperature range. The cooling curves for channels 1 and 2 (the vertically racked samples) are similar to the curves for channels 3 and 4 (the stacked samples). However, the curves for channels 1 and 2 follow different paths than the curves for channels 3 and 4, and especially so 45 in the early portion of the cooling curves (during the beginning of the cooling step).

50 Subsequently, the shapes of the curves for channels 1 and 2 reflect a faster cooling rate than for channels 3 and 4. For example, in the region of the cooling curve in which the individual channel cooling curves first intersect the CCT curve, the cooling rate for channels 1 and 2 (vertically racked samples) was approximately 136° F./min (75.6° C./min), and for channels 3 and 4 (stacked samples) were approximately 98° F./min (54.4° C./min) and approximately 107° F./min (59.4° C./min), respectively. As would be expected, the cooling rates for channels 3 and 4 fall between the cooling rates measured for the cooling trials involving two stacked plates

(111° F./min (61.7° C./min)) and 5 stacked plates (95° F./min (52.8° C./min)), discussed above. The cooling curves for the two stacked plate (“2PI”) and 5 stacked plate (“5PI”) cooling trials also are shown in FIGS. 12-14.

The cooling curves shown in FIGS. 12-14 for channels 1-4 suggest that all of the cooling rates did not substantially differ. As shown in FIGS. 12 and 13, however, each of the curves initially intersects the CCT curve at different points, indicating different amounts of transition, which may significantly affect the relative microstructures of the samples. The variation in the point of intersection of the CCT curve is largely determined by the degree of cooling that occurs while the sample is at high temperature. Therefore, the amount of cooling that occurs in the time period relatively soon after the sample is removed from the furnace may significantly affect the final microstructure of the samples, and this may in turn provide or contribute to the unexpected improvement in ballistic penetration resistance discussed herein. Therefore, the experimental trial confirmed that the manner in which the samples are cooled from the austenitizing temperature could influence alloy microstructure, and this may be at least partially responsible for the improved ballistic performance of armor alloys according to the present disclosure.

#### 5. Conventional Cooling and Tempering Tests

Ballistic test panels were prepared from an alloy having the experimental chemistry shown in Table 2 above. Alloy ingots were prepared by melting in an electric arc furnace and refined using AOD or AOD and ESR. Ingot surfaces were ground using conventional practices. The ingots were then heated to about 1300° F. (704° C.), equalized, held at this first temperature for 6 to 8 hours, heated at about 200° F./hour (93° C./hour) up to about 2050° F. (1121° C.), and held at the second temperature for about 30-40 minutes per inch of thickness. Ingots were then de-scaled and hot rolled to 6-7 inch slabs (15.2-17.8 cm). The slabs were hot sheared to form slabs

5 F. of the austenitizing temperature. The plates were removed from the furnace after 60 minutes time-at-temperature and allowed to conventionally cool in still air to room temperature. After cooling to room temperature, the plates were shot blasted to clean and descale.

10 The plates were then tempered at a temperature in the range of 250° F. to 500° F. (±5° F.) for 450 minutes to 650 minutes (±5 minutes) time-at-temperature. The tempered plates were sectioned to 12-inch by 12-inch (30.5×30.5 cm) plates having various finished gauge thicknesses in the range 0.188-0.300 inches. Six (6) 12-inch by 12-inch plates were selected for hardness testing and ballistic penetration resistance testing. The BHN of each tempered plate was determined per ASTM E-10. The  $V_{50}$  ballistic limit (protection) value for each plate was also determined per U.S. Military Specification (e.g., MIL-DTL-46100E, MIL-A-46099C, and MIL-DTL-32332) using .30 caliber M2, AP projectiles.

15 All six (6) plates were processed using generally identical methods except for the tempering temperatures and rolled finish gauges. The plate thicknesses, the tempering parameters, and the as-tempered BHN determined for each plate are provided in Table 14 and the results of the ballistic testing are provided in Table 15.

TABLE 14

| Plate    | Nominal Gauge (inches) | Average Thickness (inches) | Tempering Temperature (° F.) | Time-at-temperature (minutes) | BHN |
|----------|------------------------|----------------------------|------------------------------|-------------------------------|-----|
| 1005049A | 0.188                  | 0.192                      | 350                          | 480                           | 578 |
| 1005049B | 0.236                  | 0.240                      | 350                          | 480                           | 601 |
| 1005049C | 0.250                  | 0.254                      | 350                          | 480                           | 601 |
| 1005049G | 0.188                  | 0.195                      | 335                          | 480                           | 578 |
| 1005049H | 0.236                  | 0.237                      | 335                          | 480                           | 601 |
| 1005049I | 0.250                  | 0.252                      | 335                          | 480                           | 601 |

TABLE 15

| Plate    | Measured $V_{50}$ ballistic limit (fps) | Minimum $V_{50}$ ballistic limit per MIL-DTL-46100E (fps) | Minimum $V_{50}$ ballistic limit per MIL-A-46099C (fps) | Minimum $V_{50}$ ballistic limit per MIL-DTL-32332 (Class 1) (fps) | Minimum $V_{50}$ ballistic limit per MIL-DTL-32332 (Class 2) (fps) |
|----------|-----------------------------------------|-----------------------------------------------------------|---------------------------------------------------------|--------------------------------------------------------------------|--------------------------------------------------------------------|
| 1005049A | 2246                                    | 1765                                                      | 2280                                                    | 2103                                                               | 2303                                                               |
| 1005049B | 2565                                    | 2162                                                      | 2574                                                    | 2445                                                               | 2645                                                               |
| 1005049C | 2613                                    | 2258                                                      | 2653                                                    | 2520                                                               | 2720                                                               |
| 1005049G | 2240                                    | 1793                                                      | 2299                                                    | 2129                                                               | 2329                                                               |
| 1005049H | 2562                                    | 2140                                                      | 2557                                                    | 2428                                                               | 2628                                                               |
| 1005049I | 2703                                    | 2245                                                      | 2642                                                    | 2510                                                               | 2710                                                               |

50 having dimensions of about 6-7 inch thickness, 38-54 inch (96.5-137.2 cm) length, and 36 inch (91.4 cm) width.

The slabs were reheated to about 2050° F. (1121° C.) for 1-2 hours (time-at-temperature) before subsequent additional hot rolling to re-slabs of about 1.50-2.65 inches (3.81-6.73 cm) in thickness. The re-slabs were stress relief annealed using conventional practices. The re-slab surfaces were then blast cleaned and the edges and ends were ground.

The re-slabs were heated to about 1800° F. (982° C.) and held at temperature for 20 minutes per inch of thickness. The slabs were then finish rolled to long plates having finished gauge thicknesses ranging from about 0.188 inches (4.8 mm) to about 0.300 inch (7.6 mm).

The plates were then placed in a furnace to austenitize the constituent steel alloy by heating to a temperature in the range of 1450° F. to 1650° F. (±10° F.) for 60 minutes (±5 minutes), beginning when the surfaces of the plates reached within 10°

FIGS. 15-20 are schematic diagrams illustrating photographs of plates 1005049A-C and 1005049G-I, respectively, taken after ballistic testing per U.S. Military Specification. As shown in the diagrams illustrating the photographs, the plates did not exhibit any observable cracking or crack propagation resulting from the multiple .30 caliber AP projectile strikes. As indicated in Table 14, above, each of the plates exceeded 570 BHN, and four of the six plates exceeded 600 BHN.

60 Table 16 list the results of the ballistic testing as a difference between the measured  $V_{50}$  ballistic limit value and the minimum  $V_{50}$  ballistic limit value per U.S. Military Specification (MIL-DTL-46100E, MIL-A-46099C, and MIL-DTL-32332). For example, a value of “481” means that the  $V_{50}$  value for that particular plate exceeded the minimum required 65  $V_{50}$  limit value under the indicated U.S. Military Specification by 481 feet per second. A value of “-34” means that the  $V_{50}$  value for that particular plate was 34 feet per second less

than the minimum required  $V_{50}$  limit value under the indicated U.S. Military Specification.

the disclosed alloys at temperatures near the observable phase transition (e.g., tempering at a temperature in the range 250°

TABLE 16

| Plate    | Measured $V_{50}$ ballistic limit (fps) | Minimum $V_{50}$ per MIL-DTL-46100E (fps) | Difference Between Measured $V_{50}$ and Minimum $V_{50}$ per MIL-A-46099C (fps) | Measured $V_{50}$ and Minimum $V_{50}$ per MIL-DTL-32332 (Class 1) (fps) | Difference Between Measured $V_{50}$ and Minimum $V_{50}$ per MIL-DTL-32332 (Class 2) (fps) |
|----------|-----------------------------------------|-------------------------------------------|----------------------------------------------------------------------------------|--------------------------------------------------------------------------|---------------------------------------------------------------------------------------------|
| 1005049A | 2246                                    | 481                                       | -34                                                                              | 143                                                                      | -57                                                                                         |
| 1005049B | 2565                                    | 403                                       | -9                                                                               | 120                                                                      | -80                                                                                         |
| 1005049C | 2613                                    | 355                                       | -40                                                                              | 93                                                                       | -107                                                                                        |
| 1005049G | 2240                                    | 447                                       | -59                                                                              | 111                                                                      | -89                                                                                         |
| 1005049H | 2562                                    | 422                                       | 5                                                                                | 134                                                                      | -66                                                                                         |
| 1005049I | 2703                                    | 458                                       | 61                                                                               | 193                                                                      | -7                                                                                          |

As indicated in Table 16, each of the plates exceeded the minimum  $V_{50}$  ballistic limit values per U.S. Military Specifications MIL-DTL-46100E and MIL-DTL-32332 (Class 1). Two of the six plates exceeded the minimum  $V_{50}$  ballistic limit per MIL-A-46099C. Each of the plates exhibited a  $V_{50}$  ballistic limit value that was at least as great as a  $V_{50}$  ballistic limit value that is 150 fps less than the performance requirements under MIL-A-46099C and the Class 2 performance requirements under MIL-DTL-32332. Indeed, each of the plates exhibited a  $V_{50}$  ballistic limit value that was at least as great as a  $V_{50}$  ballistic limit value that is 60 fps less than the performance requirements under MIL-A-46099C and 110 fps less than the Class 2 performance requirements under MIL-DTL-32332.

The unexpected and surprising ballistic performance properties described above were achieved with near 600 BHN or over 600 BHN ultra-high hardness steel alloy plates that exhibited no observable cracking during the ballistic testing. These characteristics were achieved using austenitizing heat treatment, cooling to harden the alloy, and tempering treatment to toughen the alloy. It is believed that the alloying additions, for example, nickel, chromium, and molybdenum, tend to stabilize the austenite formed during the austenitizing heat treatment. The stabilization of austenite may tend to slow the transformation of the austenite to other microstructures during cooling from austenitizing temperatures. A decrease in the transformation rate of austenite may allow the formation of martensite using slower cooling rates that would otherwise tend to form microstructures rich in ferrite and cementite.

Thermal expansion measurements were conducted on an alloy having the experimental chemistry shown in Table 2 above. The thermal expansion measurements were conducted over a cooling range beginning at austenitizing temperatures (1450° F.-1650° F.) to approximately room temperature. The thermal expansion measurements revealed that at least one phase transition occurs in the alloy in the temperature range 300° F.-575° F. It is believed that the phase transition is from an austenite phase to a lower bainite phase, a lath martensite phase, or a combination of both lower bainite and lath martensite.

Generally, when an alloy having the experimental chemistry shown in Table 2 is cooled from austenitizing temperatures at a cooling rate above a threshold cooling rate (for example, in still air), the austenite phase transforms to a relatively hard twinned martensite phase and retained austenite. The retained austenite may transform to untempered twinned martensite over time. It is believed that tempering of

20 F.-500° F.) may transform the retained austenite to lower bainite and/or lath martensite. Lower bainite and lath martensite microstructures are significantly more ductile and tougher than the significantly harder twinned martensite microstructure.

25 As a result, alloys according to various embodiments of the present disclosure may have a microstructure comprising twinned martensite, lath martensite, and/or lower bainite after tempering at a temperature in the range 250° F.-500° F. This may result in steel alloys having a synergistic combination of 30 hard twinned martensite microstructure and tougher, more ductile lower bainite and/or lath martensite microstructure. A synergistic combination of hardness, toughness, and ductility may impart excellent ballistic penetration and crack resistance properties to the alloys as described herein.

35 In various embodiments, articles comprising an alloy as described herein may be heated at a temperature of 1450° F.-1650° F. to austenitize the alloy microstructure. In various embodiments, alloy articles may be heated for at least 15 minutes minimum furnace time, at least 18 minutes minimum 40 furnace time, or at least 21 minutes minimum furnace time to austenitize the alloy. In various embodiments, alloy articles may be heated for 15-60 minutes or 15-30 minutes minimum furnace time to austenitize the alloy. For example, alloy plates 45 having gauge thicknesses of 0.188-0.225 inches may be heated at a temperature of 1450° F.-1650° F. for at least 18 minutes minimum furnace time, and alloy plates having gauge thicknesses of 0.226-0.313 inches may be heated at a temperature of 1450° F.-1650° F. for at least 21 minutes minimum furnace time to austenitize the alloy. In various 50 embodiments, alloy articles may be held at 1450° F.-1650° F. for 15-60 minutes or 15-30 minutes time-at-temperature to austenitize the alloys.

55 The alloy articles may be cooled from austenitizing temperature to room temperature in still air to harden the alloy. 55 During cooling the alloy articles comprising sheets or plates may be flattened by the application of mechanical force to the article. For example, after the articles have cooled in still air to a surface temperature of 600° F. to 700° F., the plates may be flattened on a flattener/leveler apparatus. A flattening 60 operation may include the application of mechanical force to the major planar surfaces of the articles. A mechanical force may be applied, for example, using a rolling operation, a stretching operation, and/or a pressing operation. The mechanical force is applied so that the gauge thicknesses of 65 the articles are not decreased during the flattening operation. The articles are allowed to continue to cool during the flattening operation, which may be discontinued after the surface

29

temperature of the articles falls below 250° F. The articles are not stacked together until the surface temperature of the cooling articles is below 200° F.

In various embodiments, alloy articles may be tempered at a temperature in the range 250° F. to 500° F. In various embodiments, an alloy article may be tempered at a temperature in the range 300° F. to 400° F. In various embodiments, an alloy article may be tempered at a temperature in the range 325° F. to 375° F., 235° F. to 350° F., or 335° F. to 350° F., for example. In various embodiments, an alloy article may be tempered for 450-650 minutes time-at-temperature. In various embodiments, an alloy article may be tempered for 480-600 minutes time-at-temperature. In various embodiments, an alloy article may be tempered for 450-500 minutes time-at-temperature.

In various embodiments, an alloy article processed as described herein may comprise an alloy sheet or an alloy plate. In various embodiments, an alloy article may comprise an alloy plate having an average thickness of 0.118-0.630 inches (3-16 mm). In various embodiments, an alloy article may comprise an alloy plate having an average thickness of 0.188-0.300 inches. In various embodiments, an alloy article may have a hardness greater than 550, BHN, 570 BHN, or 600 BHN. In various embodiments an alloy article may have a hardness less than 700 BHN or 675 BHN. In various embodiments, an alloy article may comprise a steel armor plate.

In various embodiments, an alloy article processed as described herein may exhibit a  $V_{50}$  value that exceeds the minimum  $V_{50}$  ballistic limit value per U.S. Military Specifications MIL-DTL-46100E and MIL-DTL-32332 (Class 1). In various embodiments, an alloy article processed as described herein may exhibit a  $V_{50}$  value that exceeds the minimum  $V_{50}$  ballistic limit value per specification MIL-DTL-46100E by at least 300, at least 350, at least 400, or at least 450 fps. In various embodiments, an alloy article processed as described herein may exhibit a  $V_{50}$  value that exceeds the minimum  $V_{50}$  ballistic limit value per specification

30

may exhibit low, minimal, or zero cracking or crack propagation resulting from multiple armor piercing projectile strikes.

In various embodiments, an alloy article processed as described herein may have a microstructure comprising at least one of lath martensite and lower bainite. In various embodiments, an alloy article processed as described herein may have a microstructure comprising lath martensite and lower bainite.

#### 10 6. Processes for Making Armor Plate

The illustrative and non-limiting examples that follow are intended to further describe the various embodiments presented herein without restricting their scope. The Examples describe processes that may be utilized to make high hardness, high toughness, ballistic resistant, and crack resistant armor plates. Persons having ordinary skill in the art will appreciate that variations of the Examples are possible, for example, using different compositions, times, temperatures, and dimensions as variously described herein.

##### a. Example 1

A heat having the chemistry presented in Table 17 is prepared. Appropriate feed stock is melted in an electric arc furnace. The heat is tapped into a ladle where appropriate alloying additions are added to the melt. The heat is transferred in the ladle and poured into an AOD vessel. There the heat is decarburized using a conventional AOD operation. The decarburized heat is tapped into a ladle and poured into an ingot mold and allowed to solidify to form an ingot. The ingot is removed from the mold and may be transported to an ESR furnace where the ingot may be remelted and remolded to form a refined ingot. The ESR operation is optional and an ingot may be processed after solidification, post-AOD without ESR. The ingot has rectangular dimensions of 13×36 inches and a nominal weight of 4500 lbs.

TABLE 17

| C    | Mn   | P     | S      | Si   | Cr   | Ni   | Mo   | Ce    | La    | N     | B     |
|------|------|-------|--------|------|------|------|------|-------|-------|-------|-------|
| 0.50 | 0.50 | 0.009 | 0.0009 | 0.30 | 1.25 | 4.00 | 0.50 | 0.007 | 0.006 | 0.005 | 0.002 |

25 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760

the plates. The furnace is pre-heated to 1625° F. and the plates inserted for 21 minutes after the temperature stabilizes at 1625° F. It is believed that the plate reaches a temperature of 1600-1625° F. during the 21 minute minimum furnace time.

After completion of the 21 minute minimum furnace time, the austenitized plates are removed from the furnace and allowed to cool to 1000° F. in still air. After the plates have cooled to 1000° F., the plates are transported via an overhead crane to a Cauffiel™ flattener. After the plates have reached 600° F.-700° F., the plates are flattened on the flattener by applying mechanical force to the 54×300 inch planar surfaces of the plates. The mechanical force is applied so that the gauge thicknesses of the plates are not decreased during the flattening operation. The plates are allowed to continue to cool during the flattening operation, which is discontinued after the temperature of the plates falls below 250° F. The plates are not stacked until the temperature of the cooling plates is below 200° F.

The cooled plates are blast cleaned and sectioned to various length-by-width dimensions using an abrasive saw cutting operation. The sectioned plates are heated to 335° F. (±5° F.) in a furnace, held for 480-600 minutes (±5 minutes) at 335° F. (±5° F.) (time-at-temperature) to temper the plates, and allowed to cool to room temperature in still air. The tempered plates exhibit a hardness of at least 550 BHN.

The tempered plates find utility as armor plates exhibiting high hardness, high toughness, excellent ballistic resistance, and excellent crack resistance. The tempered plates exhibit a  $V_{50}$  ballistic limit value greater than the minimum  $V_{50}$  ballistic limit value under specification MIL-DTL-32332 (Class 1). The tempered plates also exhibit a  $V_{50}$  ballistic limit value that is at least as great as a  $V_{50}$  ballistic limit value 150 feet per second less than the required  $V_{50}$  ballistic limit value under specification MIL-DTL-32332 (Class 2).

#### b. Example 2

A heat having the chemistry present in Table 18 is prepared. Appropriate feed stock is melted in an electric arc furnace. The heat is tapped into a ladle where appropriate alloying additions are added to the melt. The heat is transferred in the ladle and poured into an AOD vessel. There the heat is decarburized using a conventional AOD operation. The decarburized heat is tapped into a ladle and poured into an ingot mold and allowed to solidify to form an ingot. The ingot is removed from the mold and may be transported to an ESR furnace where the ingot may be remelted and remolded to form a refined ingot. The ESR operation is optional and an ingot may be processed after solidification, post-AOD without ESR. The ingot has rectangular dimensions of 13×36 inches and a nominal weight of 4500 lbs.

TABLE 18

| C    | Mn   | P     | S      | Si   | Cr   | Ni   | Mo   | Ce    | La    | N     | B     |
|------|------|-------|--------|------|------|------|------|-------|-------|-------|-------|
| 0.49 | 0.20 | 0.009 | 0.0009 | 0.20 | 1.00 | 3.75 | 0.40 | 0.003 | 0.002 | 0.005 | 0.001 |

The ingot is heated in a furnace at 1300° F. for six (6) hours (minimum furnace time), after which the ingot is heated at 200° F. per hour to 2050° F. and held at 2050° F. for 30 minutes per inch of ingot thickness (13 inches, 390 minutes). The ingot is de-scaled and hot rolled at 2050° F. on a 110-inch rolling mill to form a 6×36×length inch slab. The slab is reheated in a 2050° F. furnace for 1.5 hours. The slab is hot rolled at 2050° F. on a 110-inch rolling mill to form a 1.75×36×length inch re-slab. The re-slab is hot sheared to form two (2) 1.75×36×38 inch re-slabs. The re-slabs are stress relief

annealed in a furnace using conventional practices. The re-slabs are blast cleaned, all edges and ends are ground, and the re-slabs are heated at 1800° F. for 20 minutes per inch of thickness (1.75 inches, 35 minutes).

5 The re-slabs are de-scaled and hot rolled at 1800° F. on a 110-inch rolling mill to form 0.188×54×222 inch plates. The re-slabs are re-heated to 1800° F. between passes on the rolling mill, as necessary, to avoiding finishing the rolling operation below 1425° F.

10 The 0.188×54×222 inch plates are heated in a furnace at 1600° F. for 18 minutes (minimum furnace time) to austenitize the plates. The furnace is pre-heated to 1600° F. and the plates inserted for 18 minutes after the temperature stabilizes at 1600° F. It is believed that the plate reaches a temperature of 1575-1600° F. during the 18 minute minimum furnace time.

15 After completion of the 18 minute minimum furnace time, the austenitized plates are removed from the furnace and allowed to cool to 1000° F. in still air. After the plates have cooled to 1000° F., the plates are transported via an overhead crane to a Cauffiel™ flattener. After the plates have reached 600° F.-700° F., the plates are flattened on the flattener by applying mechanical force to the 54×222 inch planar surfaces of the plates. The mechanical force is applied so that the gauge thicknesses of the plates are not decreased during the flattening operation. The plates are allowed to continue to cool during the flattening operation, which is discontinued after the temperature of the plates falls below 250° F. The plates are not stacked until the temperature of the cooling plates is below 200° F.

20 The cooled plates are blast cleaned and sectioned to various length-by-width dimensions using an abrasive saw cutting operation. The sectioned plates are heated to 325° F. (±5° F.) in a furnace, held for 480-600 minutes (±5 minutes) at 325° F. (±5° F.) (time-at-temperature) to temper the plates, and allowed to cool to room temperature in still air. The tempered plates exhibit a hardness of at least 550 BHN.

25 The tempered plates find utility as armor plates having high hardness, high toughness, excellent ballistic resistance, and excellent crack resistance. The tempered plates exhibit a  $V_{50}$  ballistic limit value greater than the minimum  $V_{50}$  ballistic limit value under specification MIL-DTL-32332 (Class 1). The tempered plates also exhibit a  $V_{50}$  ballistic limit value that is at least as great as a  $V_{50}$  ballistic limit value 150 feet per second less than the required  $V_{50}$  ballistic limit value under specification MIL-DTL-32332 (Class 2).

#### c. Example 3

A heat having the chemistry present in Table 19 is prepared. Appropriate feed stock is melted in an electric arc furnace. The heat is tapped into a ladle where appropriate

45 alloying additions are added to the melt. The heat is transferred in the ladle and poured into an AOD vessel. There the heat is decarburized using a conventional AOD operation. The decarburized heat is tapped into a ladle and poured into an ingot mold and allowed to solidify to form an ingot. The ingot is removed from the mold and may be transported to an ESR furnace where the ingot may be remelted and remolded to form a refined ingot. The ESR operation is optional and an ingot may be processed after solidification, post-AOD without ESR. The ingot has rectangular dimensions of 13×36 inches and a nominal weight of 4500 lbs.

TABLE 19

| C    | Mn   | P     | S     | Si   | Cr   | Ni   | Mo   | Ce   | La   | N     | B     |
|------|------|-------|-------|------|------|------|------|------|------|-------|-------|
| 0.51 | 0.80 | 0.010 | 0.001 | 0.40 | 1.50 | 4.25 | 0.60 | 0.01 | 0.01 | 0.007 | 0.003 |

The ingot is heated in a furnace at 1300° F. for eight (8) hours (minimum furnace time), after which the ingot is heated at 200° F. per hour to 2050° F. and held at 2050° F. for 40 minutes per inch of ingot thickness (13 inches, 520 minutes). The ingot is de-scaled and hot rolled at 2050° F. on a 110-inch rolling mill to form a 6x36xlength inch slab. The slab is reheated in a 2050° F. furnace for 1.5 hours. The slab is hot rolled at 2050° F. on a 110-inch rolling mill to form a 1.75x36xlength inch re-slab. The re-slab is hot sheared to form two (2) 1.75x36x50 inch re-slabs. The re-slabs are stress relief annealed in a furnace using conventional practices. The re-slabs are blast cleaned, all edges and ends are ground, and the re-slabs are heated to 1800° F. and held at 1800° F. for 20 minutes per inch of thickness (1.75 inches, 35 minutes).

The re-slabs are de-scaled and hot rolled at 1800° F. on a 110-inch rolling mill to form 0.250x54x222 inch plates. The re-slabs are re-heated to 1800° F. between passes on the rolling mill, as necessary, to avoiding finishing the rolling operation below 1425° F.

second less than the required  $V_{50}$  ballistic limit value under specification MIL-DTL-32332 (Class 2).

10

## d. Example 4

A heat having the chemistry present in Table 20 is prepared. Appropriate feed stock is melted in an electric arc furnace. The heat is tapped into a ladle where appropriate alloying additions are added to the melt. The heat is transferred in the ladle and poured into an AOD vessel. There the heat is decarburized using a conventional AOD operation. The decarburized heat is tapped into a ladle and poured into an ingot mold and allowed to solidify to form an 8x38x115 inch ingot. The ingot is removed from the mold and transported to an ESR furnace where the ingot is remelted and remolded to form a refined ingot. The refined ingot has rectangular dimensions of 12x42 inches and a nominal weight of 9500 lbs.

TABLE 20

| C    | Mn   | P     | S      | Si   | Cr   | Ni   | Mo   | Ce    | La    | N     | B     |
|------|------|-------|--------|------|------|------|------|-------|-------|-------|-------|
| 0.50 | 0.50 | 0.009 | 0.0009 | 0.30 | 1.25 | 4.00 | 0.50 | 0.007 | 0.006 | 0.005 | 0.002 |

The 0.250x54x222 inch plates are heated in a furnace for 21 minutes at 1625° F. (minimum furnace time) to austenitize the plates. The furnace is pre-heated to 1625° F. and the plates inserted for 21 minutes after the temperature stabilizes at 1625° F. It is believed that the plate reaches a temperature of 1600-1625° F. during the 21 minute minimum furnace time.

After completion of the 21 minute minimum furnace time, the austenitized plates are removed from the furnace and allowed to cool to 1000° F. in still air. After the plates have cooled to 1000° F., the plates are transported via overhead crane to a Cauffiel™ flattener. After the plates have reached 600° F.-700° F., the plates are flattened on the flattener by applying mechanical force to the 54x222 inch planar surfaces of the plates. The mechanical force is applied so that the gauge thicknesses of the plates are not decreased during the flattening operation. The plates are allowed to continue to cool during the flattening operation, which is discontinued after the temperature of the plates falls below 250° F. The plates are not stacked until the temperature of the cooling plates is below 200° F.

The cooled plates are blast cleaned and sectioned to various length-by-width dimensions using an abrasive saw cutting operation. The sectioned plates are heated to 350° F. ( $\pm 5$ ° F.) in a furnace, held for 480-600 minutes ( $\pm 5$  minutes) at 350° F. ( $\pm 5$ ° F.) (time-at-temperature) to temper the plates, and allowed to cool to room temperature in still air. The tempered plates exhibit a hardness of at least 550 BHN.

The tempered plates find utility as armor plates having high hardness, high toughness, excellent ballistic resistance, and excellent crack resistance. The tempered plates exhibit a  $V_{50}$  ballistic limit value greater than the minimum  $V_{50}$  ballistic limit value under specification MIL-DTL-32332 (Class 1). The tempered plates also exhibit a  $V_{50}$  ballistic limit value that is at least as great as a  $V_{50}$  ballistic limit value 150 feet per

35 inch slab. The slab is heated in a furnace at 1800° F. for one (1) hour (minimum furnace time), after which the slab is held at 1800° F. for an additional 20 minutes per inch of ingot thickness (2.7 inches, 54 additional minutes)). The slab is de-scaled and hot rolled at 1800° F. on a 110-inch rolling mill to form a 1.5x42xlength inch re-slab. The re-slab is hot sheared to form two (2) 1.5x42x48 inch re-slabs. The re-slabs are stress relief annealed in a furnace using conventional practices. The re-slabs are blast cleaned, all edges and ends are ground, and the re-slabs are heated at 1800° F. for 20 minutes per inch of thickness (1.5 inches, 30 minutes).

40 The re-slabs are de-scaled and hot rolled at 1800° F. on a 110-inch rolling mill to form 0.238x54x222 inch plates. The re-slabs are re-heated between passes on the rolling mill to 1800° F., as necessary, to avoiding finishing the rolling operation below 1425° F.

45 The 0.238x54x222 inch plates are heated in a furnace for 21 minutes at 1625° F. (minimum furnace time) to austenitize the plates. The furnace is pre-heated to 1625° F. and the plates inserted for 21 minutes after the temperature stabilizes at 1625° F. It is believed that the plate reaches a temperature of 1600-1625° F. during the 21 minute minimum furnace time.

50 After completion of the 21 minute minimum furnace time, the austenitized plates are removed from the furnace and allowed to cool to 1000° F. in still air. After the plates have cooled to 1000° F., the plates are transported via overhead crane to a Cauffiel™ flattener. After the plates have reached 600° F.-700° F., the plates are flattened on the flattener by applying mechanical force to the 54x222 inch planar surfaces of the plates. The mechanical force is applied so that the gauge thicknesses of the plates are not decreased during the flattening operation. The plates are allowed to continue to cool during the flattening operation, which is discontinued

35

after the temperature of the plates falls below 250° F. The plates are not stacked until the temperature of the cooling plates is below 200° F.

The cooled plates are blast cleaned and sectioned to various length-by-width dimensions using an abrasive saw cutting operation. The sectioned plates are heated to 335° F. (±5° F.) in a furnace, held for 480-600 minutes (±5 minutes) at 335° F. (±5° F.) (time-at-temperature) to temper the plates, and allowed to cool to room temperature in still air. The tempered plates exhibit a hardness of at least 550 BHN.

The tempered plates find utility as armor plates having high hardness, high toughness, excellent ballistic resistance, and excellent crack resistance. The tempered plates exhibit a  $V_{50}$  ballistic limit value greater than the minimum  $V_{50}$  ballistic limit value under specification MIL-DTL-32332 (Class 1). The tempered plates also exhibit a  $V_{50}$  ballistic limit value that is at least as great as a  $V_{50}$  ballistic limit value 150 feet per second less than the required  $V_{50}$  ballistic limit value under specification MIL-DTL-32332 (Class 2).

Steel armors according to the present disclosure may provide substantial value because they exhibit ballistic performance at least commensurate with premium, high alloy armor alloys, while including substantially lower levels of costly alloying ingredients such as, for example, nickel, molybdenum, and chromium. Further, steel armors according to the present disclosure exhibit ballistic performance at least commensurate with the U.S. Military Specification requirements for dual hardness, roll-bonded material, such as, for example, the requirements under described in MIL-A-46099C. Given the performance and cost advantages of embodiments of steel armors according to the present disclosure, it is believed that such armors are a very substantial advance over many existing armor alloys.

The alloy plate and other mill products made according to the present disclosure may be used in conventional armor applications. Such applications include, for example, armored sheathing and other components for combat vehicles, armaments, armored doors and enclosures, and other article of manufacture requiring or benefiting from protection from projectile strikes, explosive blasts, and other high energy insults. These examples of possible applications for alloys according to the present disclosure are offered by way of example only, and are not exhaustive of all applications to which the present alloys may be applied. Those having ordinary skill, upon reading the present disclosure, will readily identify additional applications for the alloys described herein. It is believed that those having ordinary skill in the art will be capable of fabricating all such articles of manufacture from alloys according to the present disclosure based on knowledge existing within the art. Accordingly, further discussion of fabrication procedures for such articles of manufacture is unnecessary here.

The present disclosure has been written with reference to various exemplary, illustrative, and non-limiting embodiments. However, it will be recognized by persons having ordinary skill in the art that various substitutions, modifications, or combinations of any of the disclosed embodiments (or portions thereof) may be made without departing from the scope of the invention as defined solely by the claims. Thus, it is contemplated and understood that the present disclosure embraces additional embodiments not expressly set forth herein. Such embodiments may be obtained, for example, by combining, modifying, or reorganizing any of the disclosed steps, ingredients, constituents, components, elements, features, aspects, and the like, of the embodiments described herein. Thus, this disclosure is not limited by the description of the various exemplary, illustrative, and non-limiting

36

embodiments, but rather solely by the claims. In this manner, Applicants reserve the right to amend the claims during prosecution to add features as variously described herein.

What is claimed is:

1. A process for making an alloy article comprising: austenitizing an alloy article by heating the alloy article at a temperature of at least 1450° F. for at least 15 minutes minimum furnace time, the alloy comprising, in weight percentages based on total alloy weight:
  - 10 0.40 to 0.53 carbon;
  - 0.15 to 1.00 manganese;
  - 0.15 to 0.45 silicon;
  - 0.95 to 1.70 chromium;
  - 3.30 to 4.30 nickel;
  - 0.35 to 0.65 molybdenum;
  - 0.0002 to 0.0050 boron;
  - 0.001 to 0.015 cerium;
  - 0.001 to 0.015 lanthanum;
  - no greater than 0.002 sulfur;
  - no greater than 0.015 phosphorus;
  - no greater than 0.011 nitrogen;
  - iron; and
  - incidental impurities;
 cooling the alloy article from the austenitizing temperature in still air; and
 tempering the alloy article at a temperature of 250° F. to 500° F. for 450 minutes to 650 minutes time-at-temperature, directly after the cooling in still air, thereby providing a tempered alloy article exhibiting a hardness greater than 570 BHN.
2. The process of claim 1, comprising tempering the alloy article at a temperature of 325° F. to 350° F. for 480 minutes to 600 minutes time-at-temperature, thereby providing a tempered alloy article.
3. The process of claim 1, wherein the tempered alloy article exhibits a hardness greater than 570 BHN and less than 675 BHN.
4. The process of claim 1, wherein the tempered alloy article exhibits a hardness greater than 600 BHN and less than 675 BHN.
5. The process of claim 1, wherein the tempered alloy article exhibits a  $V_{50}$  ballistic limit value greater than the minimum  $V_{50}$  ballistic limit value under specification MIL-DTL-32332 (Class 1).
- 45 6. The process of claim 1, wherein the tempered alloy article exhibits a  $V_{50}$  ballistic limit value that exceeds the minimum  $V_{50}$  ballistic limit value under specification MIL-DTL-32332 (Class 1) by at least 50 feet per second.
7. The process of claim 1, wherein the tempered alloy article exhibits a  $V_{50}$  ballistic limit value that is at least as great as a  $V_{50}$  ballistic limit 150 feet per second less than the required  $V_{50}$  ballistic limit under specification MIL-DTL-32332 (Class 2).
8. The process of claim 1, wherein the tempered alloy article exhibits a  $V_{50}$  ballistic limit value that is at least as great as a  $V_{50}$  ballistic limit 100 feet per second less than the required  $V_{50}$  ballistic limit under specification MIL-DTL-32332 (Class 2).
- 55 9. The process of claim 1, wherein the tempered alloy article exhibits zero observable cracking when subjected to a .30 caliber M2, AP projectile strike.
10. The process of claim 1, wherein the tempered alloy article has a microstructure comprising at least one of lath martensite phase and lower bainite phase.
- 60 11. The process of claim 1, wherein the tempered alloy article comprises a plate having a thickness in the range of 0.188-0.300 inches.

12. The process of claim 1, wherein the tempered alloy article comprises an armor plate or an armor sheet.

13. The process of claim 1, wherein the alloy comprises:

0.49 to 0.51 carbon;

0.2 to 0.8 manganese;

0.2 to 0.40 silicon;

1.00 to 1.50 chromium;

3.75 to 4.25 nickel;

0.40 to 0.60 molybdenum;

0.0010 to 0.0030 boron;

0.003 to 0.010 cerium; and

0.002 to 0.010 lanthanum.

5

10

\* \* \* \* \*